



US005589277A

**United States Patent** [19]**Malhotra**[11] **Patent Number:** **5,589,277**[45] **Date of Patent:** **\*Dec. 31, 1996**[54] **RECORDING SHEETS CONTAINING AMINO ACIDS, HYDROXY ACIDS, AND POLYCARBOXYL COMPOUNDS**[75] Inventor: **Shadi L. Malhotra**, Mississauga, Canada[73] Assignee: **Xerox Corporation**, Stamford, Conn.

[\*] Notice: The term of this patent shall not extend beyond the expiration date of Pat. No. 5,451,466.

[21] Appl. No.: **196,679**[22] Filed: **Feb. 15, 1994**[51] **Int. Cl.<sup>6</sup>** ..... **B41M 5/00**[52] **U.S. Cl.** ..... **428/500**; 428/195; 428/203; 428/211; 428/511; 428/537.5[58] **Field of Search** ..... 428/195, 537.5, 428/500, 511, 203, 211[56] **References Cited**

## U.S. PATENT DOCUMENTS

|           |         |                 |         |
|-----------|---------|-----------------|---------|
| 4,446,174 | 5/1984  | Mackawa et al.  | 427/261 |
| 4,554,181 | 11/1985 | Cousin et al.   | 427/261 |
| 4,576,867 | 3/1986  | Miyamoto et al. | 428/342 |
| 4,624,985 | 11/1986 | Tsutsumi et al. | 524/803 |
| 4,740,420 | 4/1988  | Akutsu et al.   | 428/341 |
| 4,775,594 | 10/1988 | Desjarlais      | 428/421 |
| 4,781,985 | 11/1988 | Desjarlais      | 428/421 |
| 4,830,911 | 5/1989  | Kojima et al.   | 428/342 |
| 4,877,680 | 10/1989 | Sakaki et al.   | 428/332 |
| 4,946,741 | 8/1990  | Aono et al.     | 428/336 |

|           |         |                 |         |
|-----------|---------|-----------------|---------|
| 5,073,448 | 12/1991 | Viera et al.    | 428/331 |
| 5,212,008 | 5/1993  | Malhotra et al. | 428/216 |
| 5,219,687 | 6/1993  | Suzuki et al.   | 430/49  |
| 5,220,346 | 6/1993  | Carrura et al.  | 346/1.1 |
| 5,223,338 | 6/1993  | Malhotra        | 428/342 |
| 5,451,458 | 9/1995  | Malhotra        | 428/195 |
| 5,451,466 | 9/1995  | Malhotra        | 428/195 |

## FOREIGN PATENT DOCUMENTS

|           |        |                    |   |
|-----------|--------|--------------------|---|
| 0439363   | 3/1991 | European Pat. Off. | . |
| 62-85982  | 4/1987 | Japan.             | . |
| 63-209884 | 8/1988 | Japan.             | . |
| 63-205276 | 8/1988 | Japan.             | . |
| 9246107   | 6/1992 | South Africa.      | . |

## OTHER PUBLICATIONS

WOA01938 (Minnesota Mining and Manufacturing Company 1-5, 7-11.

Product #: T34223 Name DL-Threonine, 99% Material Safety Data Sheet, Valid Aug. 1995-Oct. 1995.

Primary Examiner—Pamela R. Schwartz  
Attorney, Agent, or Firm—Judith L. Byorick[57] **ABSTRACT**

Disclosed is a recording sheet which comprises a paper substrate and a material selected from the group consisting of monomeric amino acids, monomeric hydroxy acids, monomeric polycarboxyl compounds, and mixtures thereof. Another embodiment of the present invention is directed to a recording sheet which comprises a substrate and a material selected from the group consisting of monomeric amino acids, monomeric hydroxy acids, and mixtures thereof.

**36 Claims, No Drawings**

RECORDING SHEETS CONTAINING AMINO  
ACIDS, HYDROXY ACIDS, AND  
POLYCARBOXYL COMPOUNDS

5

BACKGROUND OF THE INVENTION

The present invention is directed to recording sheets, such as transparency materials, filled plastics, papers, and the like. More specifically, the present invention is directed to recording sheets particularly suitable for use in ink jet printing processes. One embodiment of the present invention is directed to a recording sheet which comprises a paper substrate and a material selected from the group consisting of monomeric amino acids, monomeric hydroxy acids, monomeric polycarboxyl compounds, and mixtures thereof. Another embodiment of the present invention is directed to a recording sheet which comprises a substrate and a material selected from the group consisting of monomeric amino acids, monomeric hydroxy acids, and mixtures thereof.

Recording sheets suitable for use in ink jet printing are known. For example, U.S. Pat. No. 4,740,420 (Akutsu et al.) discloses a recording medium for ink jet printing comprising a support material containing at least in the surface portion thereof a water soluble metal salt with the ion valence of the metal thereof being 2 to 4 and a cationic organic material. The cationic organic materials include salts of alkylamines, quaternary ammonium salts, polyamines, and basic latexes.

U.S. Pat. No. 4,576,867 (Miyamoto) discloses an ink jet recording paper with improved water resistance and sunlight fastness of the image formed on the paper wherein the recording paper has attached to its surface a cationic resin of the formula



wherein  $\text{R}_1$ ,  $\text{R}_2$ , and  $\text{R}_3$  represent alkyl groups,  $m$  represents a number of 1 to 7, and  $n$  represents a number of 2 to 20, and  $\text{Y}$  represents an acid residue.

U.S. Pat. No. 4,446,174 (Maekawa et al.) discloses an ink jet recording method for producing a recorded image on an image receiving sheet with a jet of aqueous ink, wherein an ink jet is projected onto an image receiving sheet comprising a surface layer containing a pigment, and wherein the surface layer is capable of adsorbing a coloring component in the aqueous ink. Poly (vinyl benzyl trimethyl ammonium chloride), poly (diallyl dimethyl ammonium chloride), and poly (methacryloxyethyl- $\beta$ -hydroxyethyl dimethyl ammonium chloride) are disclosed as dye absorbing adhesive materials.

U.S. Pat. No. 4,830,911 (Kojima et al.) discloses a recording sheet for ink jet printers which gives an image by the use of an aqueous ink containing a water-soluble dye, coated or impregnated with either of or a mixture of two kinds of water soluble polymers, one whose polymeric unit is alkylquaternaryammonium (meth)acrylate and the other whose polymer unit is alkylquaternaryammonium (meth)acrylamide, wherein the water soluble polymers contain not less than 50 mol percent of a monomer represented by the formula



where  $\text{R}$  represents hydrogen or methyl group,  $n$  is an integer from 1 to 3 inclusive,  $\text{R}_1$ ,  $\text{R}_2$ , and  $\text{R}_3$  represent hydrogen or the same or different aliphatic alkyl group with 1 to 4 carbon atoms,  $\text{X}$  represents an anion such as a halogen ion, sulfate ion, alkyl sulfate ion, alkyl sulfonate ion, aryl sulfonate ion, and acetate ion, and  $\text{Y}$  represents oxygen or imino group.

U.S. Pat. No. 4,554,181 (Cousin et al.) discloses an ink jet recording sheet having a recording surface which includes a combination of a water soluble polyvalent metal salt and a cationic polymer, the polymer having cationic groups which are available in the recording surface for insolubilizing an anionic dye.

U.S. Pat. No. 4,877,680 (Sakaki et al.) discloses a recording medium comprising a substrate and a nonporous ink receiving layer. The ink receiving layer contains a water-insoluble polymer containing a cationic resin. The recording medium may be employed for recording by attaching droplets of a recording liquid thereon.

European Patent Publication 0 439 363 A1, published Jul. 31, 1991, corresponding to U.S. Pat. No. 5,302,249, the disclosure of which is totally incorporated herein by reference, discloses a paper which comprises a supporting substrate with a coating comprising (a) a desizing component selected from the group consisting of (1) hydrophilic poly(dialkylsiloxanes); (2) poly(alkylene glycol); (3) poly(propylene oxide)—poly(ethylene oxide) copolymers; (4) fatty ester modified compounds of phosphate, sorbitan, glycerol, poly(ethylene glycol), sulfosuccinic acid, sulfonic acid and alkyl amine; (5) poly(oxyalkylene) modified compounds of sorbitan esters, fatty amines, alkanol amides, castor oil, fatty acids and fatty alcohols; (6) quaternary alkylsulfate compounds; (7) fatty imidazolines; and mixtures thereof, and (b) a hydrophilic binder polymer. The binder polymer may be a quaternary ammonium copolymer such as Mirapol WT, Mirapol AD-1, Mirapol AZ-1, Mirapol A-15, Mirapol-9, Merquat-100, or Merquat-550, available from Miranol Incorporated.

U.S. Pat. No. 5,223,338 (Malhotra), the disclosure of which is totally incorporated herein by reference, discloses a recording sheet which comprises a substrate and a coating consisting essentially of (1) quaternary ammonium polymers selected from the group consisting of (a) polymers of Formula I



wherein  $n$  is an integer of from 1 to about 200,  $\text{R}_1$ ,  $\text{R}_2$ ,  $\text{R}_3$ , and  $\text{R}_4$  are each independently selected from the group consisting of alkyl groups, hydroxyalkyl groups, and polyoxyalkylene groups,  $p$  is an integer of from 1 to about 10,  $q$  is an integer of from 1 to about 10,  $\text{X}$  is an anion, and  $\text{Y}_1$  is selected from the group consisting of  $-\text{CH}_2\text{CH}_2\text{OCH}_2\text{CH}_2-$ ,

—CH<sub>2</sub>CH<sub>2</sub>OCH<sub>2</sub>CH<sub>2</sub>OCH<sub>2</sub>CH<sub>2</sub>—, —(CH<sub>2</sub>)<sub>k</sub>—, wherein k is an integer of from about 2 to about 10, and —CH<sub>2</sub>CH(OH)CH<sub>2</sub>—; (b) polymers of Formula II



wherein wherein n is an integer of from 1 to about 200, R<sub>5</sub>, R<sub>6</sub>, R<sub>7</sub>, and R<sub>8</sub> are each independently selected from the group consisting of alkyl groups, hydroxyalkyl groups, and polyoxyalkylene groups, m is an integer of from 0 to about 40, r is an integer of from 1 to about 10, s is an integer of from 1 to about 10, X is an anion, and Y<sub>2</sub> is selected from the group consisting of —CH<sub>2</sub>CH<sub>2</sub>OCH<sub>2</sub>CH<sub>2</sub>—, —CH<sub>2</sub>CH<sub>2</sub>OCH<sub>2</sub>CH<sub>2</sub>OCH<sub>2</sub>CH<sub>2</sub>—, —(CH<sub>2</sub>)<sub>k</sub>—, wherein k is an integer of from about 2 to about 10, and —CH<sub>2</sub>CH(OH)CH<sub>2</sub>—; (c) copolymers of Formula III



wherein a and b are each integers wherein the sum of a+b is from about 2 to about 200, R<sub>1</sub>, R<sub>2</sub>, R<sub>3</sub>, R<sub>4</sub>, R<sub>5</sub>, R<sub>6</sub>, R<sub>7</sub>, and R<sub>8</sub> are each independently selected from the group consisting of alkyl groups, hydroxyalkyl groups, and polyoxyalkylene groups, p is an integer of from 1 to about 10, q is an integer of from 1 to about 10, X is an anion, and Y<sub>1</sub> and Y<sub>2</sub> are each independently selected from the group consisting of —CH<sub>2</sub>CH<sub>2</sub>OCH<sub>2</sub>CH<sub>2</sub>—, —CH<sub>2</sub>CH<sub>2</sub>OCH<sub>2</sub>CH<sub>2</sub>OCH<sub>2</sub>CH<sub>2</sub>—, —(CH<sub>2</sub>)<sub>k</sub>—, wherein k is an integer of from about 2 to about 10, and —CH<sub>2</sub>CH(OH)CH<sub>2</sub>—; (d) mixtures of polymers of Formula I and polymers of Formula II; (e) mixtures of polymers of Formula I and copolymers of Formula III; (f) mixtures of polymers of Formula II and copolymers of Formula III; and (g) mixture of polymers of Formula I, polymers of Formula II, and copolymers of Formula III; (2) an optional binder polymer; and (3) an optional filler.

U.S. Pat. No. 5,212,008 (Malhotra et al.), the disclosure of which is totally incorporated herein by reference, discloses a recording sheet which comprises a substrate; a first coating in contact with the substrate which comprises a crosslinking agent selected from the group consisting of hexamethoxymethyl melamine, methylated melamine-formaldehyde, methylated urea-formaldehyde, cationic urea-formaldehyde, cationic polyamine-epichlorohydrin, glyoxal-urea resin, poly (aziridine), poly (acrylamide), poly (N,N-dimethyl acrylamide), acrylamide-acrylic acid copolymer, poly (2-acrylamido-2-methyl propane sulfonic acid), poly (N,N-dimethyl-3,5-dimethylene piperidinium chloride), poly (methylene-guanidine) hydrochloride, poly (ethylene imine) poly (ethylene imine) epichlorohydrin, poly (ethylene imine) ethoxylated, glutaraldehyde, and mixtures thereof; a catalyst; and a polymeric material capable of being crosslinked by the crosslinking agent and selected from the group consisting of polysaccharides having at least one hydroxy group, polysaccharides having at least one carboxy group, polysaccharides having at least one sulfate group, polysaccharides having at least one amine or amino group, polysaccharide gums, poly (alkylene oxides), vinyl polymers, and mixtures thereof; and a second coating in contact with the first coating which comprises a binder and a material selected from the group consisting of fatty imida-

zolines, ethosulfate quaternary compounds, dialkyl dimethyl methosulfate quaternary compounds, alkoxyated di-fatty quaternary compounds, amine oxides, amine ethoxylates,

10 Imidazoline quaternary compounds, alkyl benzyl dimethyl quaternary compounds, poly (epiamines), and mixtures thereof.

15 U.S. Pat. No. 4,946,741 (Aono et al.) discloses an ink recording sheet comprising a transparent support having thereon an ink recording layer comprising a mixture of an amino group deactivated gelatin derivative and a polyalkylene oxide.

U.S. Pat. No. 4,781,985 (Desjarlais) discloses an ink jet transparency which comprises a substantially transparent



resinous support and a substantially clear coating thereon which includes a specific fluorosurfactant.

30 U.S. Pat. No. 5,073,448 (Vieira et al.) discloses a recording material for ink jet printing comprising a carrier having a surface which can be printed on or a carrier coated on one side with a material which can be printed on, wherein the carrier or the coting contains as a stabilizer at least one compound of the formula



35 40 45 in which R<sub>1</sub> and R<sub>2</sub> independently of one another are C<sub>1</sub>—C<sub>4</sub> alkyl which is unsubstituted or substituted by one or two —OH, —COO—M+ and/or —SO<sub>3</sub><sup>—</sup>M+ groups, C<sub>3</sub>—C<sub>5</sub> alk- enyl, C<sub>3</sub>—C<sub>5</sub> alkynyl,



55 60 65 —CH<sub>2</sub>CH(OH)CH<sub>2</sub>—SO<sub>3</sub><sup>—</sup>M+, —CO-alkyl(C<sub>1</sub>—C<sub>4</sub>) which is unsubstituted or substituted by —COOR' or —CO—N(R<sub>5</sub>)(R<sub>6</sub>) or, if OR<sub>1</sub> and OR<sub>2</sub> are in the ortho position relative to one another, R<sub>1</sub> and R<sub>2</sub> together are C<sub>1</sub>—C<sub>6</sub> alkylene, M+ being H+, a monovalent, divalent or trivalent metal cation or a group (R<sub>12</sub>')N+(R<sub>12</sub>'')(R<sub>13</sub>')(R<sub>14</sub>''), wherein R<sub>12</sub>', R<sub>12</sub>'', R<sub>13</sub> and R<sub>14</sub> independently of one another are H, C<sub>1</sub>—C<sub>4</sub> alkyl which is unsubstituted or substituted by 1 or 3 OH, C<sub>1</sub>—C<sub>4</sub> alkyl interrupted by O, allyl, cyclopentyl, cyclohexyl, phenyl, benzyl or tolyl, or R<sub>1</sub> is a group



5

in which  $p'$  is a number from 2 to 6,  $R_5$  and  $R_6$  independently of one another are H or  $C_1-C_4$  alkyl which is unsubstituted or substituted by an OH,  $COOR'$ ,  $-COO-M+$ ,  $SO_3-M+$ ,  $P(O)(O-M+)_2$  or  $P(O)(OR')_2$  group,  $R_3'$  and  $R_4'$  independently of one another are H,  $C_1-C_4$  alkyl, OH or  $C_1-C_4$  alkoxy,  $R_3$  and  $R_4$  independently of one another are H, halogen,  $-OR_7$ ,  $-COOR'$ ,  $-COO-M+$ ,  $-OOC-R_5$ ,  $-CO-N(R_5)(R_6)$ ,  $-(R_5)N-CO-R_6$ ,  $-CO-R_5$ ,  $-SO_3-M+$ ,  $-SO_2N(R_5)(R_6)$ ,  $P(OR_5)_3$ ,  $-(O)P-(O-M+)_2$ ,  $-(O)P-(OR')_2$ ,  $C_1-C_8$  alkyl which is unsubstituted or substituted by 1 to 7  $-OR_5$  or  $-OO-C-R_5$  groups, by 1 or 2  $-COOR'$ ,  $-COO-M+$ , or  $-CO-N(R_5)(R_6)$  groups or by one or two  $-SO_3-M+$ ,  $-SO_2N(R_5)(R_6)$  or  $-(O)P-(OR')_2$  or  $-(O)P(O-M+)_2$  groups, where  $M+$ ,  $R_5$  and  $R_6$  are as defined above, or  $C_5-C_6$  cycloalkyl or allyl,  $R'$  being  $C_1-C_4$  alkyl which is unsubstituted or substituted by an OH group or  $-(CH_2CH_2O)_r-H$  in which  $r$  is 1 to 12, and  $R_7$  being  $C_1-C_4$  alkyl or  $-CO$ -alkyl( $C_1-C_4$ ) each of which is unsubstituted or substituted by 1 or 2 OH groups or  $R_3$  and  $R_4$  independently of one another are one of the groups



and  $R_{16}$  is one of the following radicals:



in which  $R_{25}$  is H or  $C_1-C_4$  alkyl,  $R_{17}$  is H,  $C_1-C_4$  alkyl which is unsubstituted or substituted by an OH group,  $-CH_2-CH(OH)-CH_2-OH$ ,  $C_1-C_4$  alkoxy, OH,  $-CO$ -alkyl( $C_1-C_4$ ),  $-COCH=CH_2$ , allyl, benzyl or a group



35

in which  $s$  is the number 2 or 3,  $t$  is a number from 0 to 2 and  $R_{21}$  and  $R_{22}$  independently of one another are H,  $C_1-C_4$  alkyl or phenyl.

South African Patent Application 924,610 discloses a transparent recording sheet suitable for making visual transparencies which comprises a thin transparent film backing bearing on at least one major surface thereof an ink jet receptive layer comprising from 1% to 10% of at least one acid having a  $pK_a$  of from 2 to 6, said acid being selected from the group consisting of aryl monocarboxylic acids, aryloxy monocarboxylic acids, alkyl carboxylic acids having alkyl groups containing at least 11 carbon atoms, dicarboxylic acids, tricarboxylic acids, and pyridinium salts, and at least one liquid-absorbent polymer comprising from 90% to 99% aprotic constituents, wherein said sheet shows reduced fading when imaged with an ink containing triaryl-methane dye and at least one nucleophile over an identical composition containing no protic organic-solvent-soluble additive.

U.S. Pat. No. 5,220,346 (Carreira et al.), the disclosure of which is totally incorporated herein by reference, discloses a printing process which comprises applying in imagewise fashion to a substrate an ink composition which comprises an aqueous liquid vehicle, a colorant, and an ionic compound at least partially ionizable in the liquid vehicle, said ink composition having a conductivity of at least about 10 milliSiemens per centimeter, and subsequently exposing the substrate to microwave radiation, thereby drying the images on the substrate. A specific embodiment of the invention is directed to a thermal ink jet printing process which comprises (1) incorporating into a thermal ink jet printing apparatus an ink composition which comprises an aqueous

in which  $R_8$  is a direct bond or methylene,  $R_9$  is H,  $C_1-C_4$  alkyl,  $-COO-M+$  or  $-SO_3-M+$ , where  $M+$ ,  $R_1$  and  $R_2$  are as defined above,  $R_{15}$  is  $-CO-$ ,  $-(O)_g-C_p'H_{2p}-$ ,  $CO-$ ,  $-OOC-C_p'H_{2p}-$ ,  $-COO-C_p'H_{2p}-$ ,  $-O-CH_2CH(OH)-CH_2-$  or



in which  $g$  is 0 or 1 and  $p$  is 1 to 6 and  $R_{24}$  is  $-OR_5$ ,  $-N(R_5)(R_6)$  or a group

liquid vehicle, a colorant, and an ionic compound at least partially ionizable in the liquid vehicle, said ink composition having a conductivity of at least about 10 millisiemens per centimeter; (2) heating the ink in an imagewise pattern to cause bubbles to form therein, thereby causing droplets of the ink to be ejected in an imagewise pattern onto a substrate, thereby generating images on the substrate; and (3) exposing the substrate to microwave radiation, thereby drying the images on the substrate.

Copending application U.S. Ser. No. 08/034,917, with the named inventors Shadi L. Malhotra, Brent S. Bryant, and Doris K. Weiss, filed Mar. 19, 1993, entitled "Recording Sheets Containing Phosphonium Compounds," the disclosure of which is totally incorporated herein by reference, discloses a recording sheet which comprises a base sheet, a phosphonium compound, an optional pigment, and an optional binder. In a preferred embodiment, the phosphonium compound is selected from the group consisting of



wherein R is an alkyl group, X is an anion, and all four R groups are the same;



wherein R is an alkyl group, wherein all three R groups are the same, wherein R is not the same as R', X is an anion, and R' is selected from the group consisting of alkyl groups, substituted alkyl groups, arylalkyl groups, and substituted arylalkyl groups;



wherein Ar is an aryl group or a substituted aryl group, X is an anion, and all four Ar groups are the same;



wherein Ar is an aryl group or a substituted aryl group, wherein all three Ar groups are the same, X is an anion, and R' is selected from the group consisting of alkyl groups, substituted alkyl groups, arylalkyl groups, and substituted arylalkyl groups; and mixtures thereof.

Copending application U.S. Pat. No. 5,314,747, with the named inventors Shadi L. Malhotra and Brent S. Bryant, filed Mar. 19, 1993, entitled "Recording Sheets Containing Cationic Sulfur Compounds," the disclosure of which is totally incorporated herein by reference, discloses a recording sheet which comprises (a) a base sheet; (b) a cationic sulfur compound selected from the group consisting of sulfonium compounds, thiazolium compounds, benzothiazolium compounds, and mixtures thereof; (c) an optional binder; and (d) an optional pigment.

Copending application U.S. Pat. No. 5,441,795, with the named inventors Shadi L. Malhotra and Brent S. Bryant, filed March 19, 1993, entitled "Recording Sheets Containing Pyridinium Compounds," the disclosure of which is totally incorporated herein by reference, discloses a recording sheet which comprises a base sheet and a material selected from

5

10

15

20

25

30

35

40

45

50

55

60

65

the group consisting of pyridinium compounds, piperazinium compounds, and mixtures thereof.

Copending application U.S. Pat. No. 5,320,902, with the named inventors Shadi L. Malhotra, Brent S. Bryant, and Doris K. Weiss, filed March 19, 1993, entitled "Recording Sheets Containing Monoammonium Compounds," the disclosure of which is totally incorporated herein by reference, discloses a recording sheet which consists essentially of a substrate and, in contact with the substrate, a monoammonium compound of the formula:



I

wherein R is an alkyl group, X is selected from the group consisting of fluoride, chloride, bromide, iodide, and astatide, and R', R'', and R''' are each independently selected from the group consisting of alkyl groups, substituted alkyl groups, aryl groups, substituted aryl groups, arylalkyl groups, and substituted arylalkyl groups, wherein R, R', R'' and R''' are either the same as or different from each other; and mixtures thereof; an optional binder component; and an optional filler component.

Copending application U.S. Pat. No. 5,457,486, with the named inventors Shadi L. Malhotra, Brent S. Bryant, and Doris K. Weiss, filed Mar. 19, 1993, entitled "Recording Sheets Containing Tetrazolium, Indolinium, and Imidazolinium Compounds," the disclosure of which is totally incorporated herein by reference, discloses a recording sheet which comprises (a) a base sheet; (b) a material selected from the group consisting of tetrazolium compounds, indolinium compounds, imidazolinium compounds, and mixtures thereof; (c) an optional pigment; and (d) an optional binder.

Copending application U.S. Pat. No. 5,550,668, with the named inventors Shadi L. Malhotra, Kurt B. Gundlach, and Richard L. Colt, filed concurrently herewith, entitled "Recording Sheets for Printing Processes Using Microwave Drying," the disclosure of which is totally incorporated herein by reference, discloses a printing process which comprises (a) providing a recording sheet which comprises a substrate, at least one monomeric salt, an optional binder, an optional antistatic agent, an optional biocide, and an optional filler; (b) applying an aqueous recording liquid to the recording sheet in an imagewise pattern; and (c) thereafter exposing the substrate to microwave radiation, thereby drying the recording liquid on the recording sheet.

Copending application U.S. Ser. No. 08/196,607, with the named inventor Shadi L. Malhotra, filed concurrently herewith, entitled "Recording Sheets Containing Alcohols and Saccharides," the disclosure of which is totally incorporated herein by reference, discloses a recording sheet which comprises a substrate and a material selected from the group consisting of monosaccharides, oligosaccharides, and mixtures thereof. Another embodiment of the present invention is directed to a printing process which comprises (a) providing a recording sheet which comprises a substrate, a material selected from the group consisting of monomeric alcohols, monosaccharides, oligosaccharides, and mixtures thereof, an optional binder, an optional antistatic agent, an optional biocide, and an optional filler; (b) applying an aqueous recording liquid to the recording sheet in an imagewise pattern; and (c) thereafter exposing the substrate to microwave radiation, thereby drying the recording liquid on the recording sheet.

Copending application U.S. Ser. No. 08/196,607, with the named inventor Shadi L. Malhotra, filed concurrently here-

with, entitled "Recording Sheets Containing Amine Salts and Quaternary Choline Halides," the disclosure of which is totally incorporated herein by reference, discloses a recording sheet which comprises a substrate and a material selected from the group consisting of monomeric amine acid salts, monomeric quaternary choline halides, and mixtures thereof.

Copending application U.S. Ser. No. 08/196,676, with the named inventor Shadi L. Malhotra, filed concurrently herewith, entitled "Recording Sheets Containing Pyrrole, Pyrrolidine, Pyridine, Piperidine, Homopiperidine, Quinoline, Isoquinoline, Quinuclidine, Indole, and Indazole Compounds," the disclosure of which is totally incorporated herein by reference, discloses a recording sheet which comprises a substrate and an additive material selected from the group consisting of pyrrole compounds, pyrrolidine compounds, pyridine compounds, piperidine compounds, homopiperidine compounds, quinoline compounds, isoquinoline compounds, quinuclidine compounds, indole compounds, indazole compounds, and mixtures thereof.

Copending application U.S. Ser. No. 08/196,933, with the named inventor Shadi L. Malhotra, filed concurrently herewith, entitled "Recording Sheets Containing Purine, Pyrimidine, Benzimidazole, Imidazolidine, Urazole, Pyrazole, Triazole, Benzotriazole, Tetrazole, and Pyrazine Compounds," the disclosure of which is totally incorporated herein by reference, discloses a recording sheet which comprises a substrate and a material selected from the group consisting of purine compounds, pyrimidine compounds, benzimidazole compounds, imidazolidine compounds, urazole compounds, pyrazole compounds, triazole compounds, benzotriazole compounds, tetrazole compounds, pyrazine compounds, and mixtures thereof. Also disclosed is a recording sheet which consists essentially of a substrate, at least one material selected from the group consisting of purine compounds, pyrimidine compounds, benzimidazole compounds, imidazolidine compounds, urazole compounds, pyrazole compounds, triazole compounds, benzotriazole compounds, tetrazole compounds, pyrazine compounds, and mixtures thereof, an optional binder, an optional antistatic agent, an optional biocide, and an optional filler.

Copending application U.S. Ser. No. 08/196,672, with the named inventor Shadi L. Malhotra, filed concurrently herewith, entitled "Recording Sheets Containing Oxazole, Isooxazole, Oxazolidinone, Oxazoline Salt, Morpholine, Thiazole, Thiazolidine, Thiadiazole, and Phenothiazine Compounds," the disclosure of which is totally incorporated herein by reference, discloses a recording sheet which comprises a substrate and a material selected from the group consisting of oxazole compounds, isoxxazole compounds, oxazolidinone compounds, oxazoline salt compounds, morpholine compounds, thiazole compounds, thiazolidine compounds, thiadiazole compounds, phenothiazine compounds, and mixtures thereof. Also disclosed is a recording sheet which consists essentially of a substrate, at least one material selected from the group consisting of oxazole compounds, isoxxazole compounds, oxazolidinone compounds, oxazoline salt compounds, morpholine compounds, thiazole compounds, thiazolidine compounds, thiadiazole compounds, phenothiazine compounds, and mixtures thereof, an optional binder, an optional antistatic agent, an optional biocide, and an optional filler.

Copending application U.S. Ser. No. 08/196,605, with the named inventors Shadi L. Malhotra, Brent S. Bryant, and Arthur Y. Jones, filed concurrently herewith, entitled "Recording Sheets Containing Mildew Preventing Agents," the disclosure of which is totally incorporated herein by

reference, discloses a recording sheet which comprises a substrate, an image receiving coating, and a biocide.

While known compositions and processes are suitable for their intended purposes, a need remains for improved recording sheets. In addition, there is a need for improved recording sheets suitable for use in ink jet printing processes. Further, a need remains for recording sheets which exhibit rapid drying times when imaged with aqueous inks. Additionally, there is a need for recording sheets which enable precipitation of a dye from a liquid ink onto the sheet surface during printing processes. A need also remains for recording sheets which are particularly suitable for use in printing processes wherein the recorded substrates are imaged with liquid inks and dried by exposure to microwave radiation. Further, there is a need for recording sheets coated with a discontinuous, porous film. There is also a need for recording sheets which, subsequent to being imaged with an aqueous ink, exhibit reduced curling.

## 20 SUMMARY OF THE INVENTION

It is an object of the present invention to provide recording sheets with the above noted advantages.

It is another object of the present invention to provide recording sheets suitable for use in ink jet printing processes.

It is yet another object of the present invention to provide recording sheets which exhibit rapid drying times when imaged with aqueous inks.

It is still another object of the present invention to provide recording sheets which enable precipitation of a dye from a liquid ink onto the sheet surface during printing processes.

Another object of the present invention is to provide recording sheets which are particularly suitable for use in printing processes wherein the recorded substrates are imaged with liquid inks and dried by exposure to microwave radiation.

Yet another object of the present invention is to provide recording sheets coated with a discontinuous, porous film.

Still another object of the present invention is to provide recording sheets which, subsequent to being imaged with an aqueous ink, exhibit reduced curling.

These and other objects of the present invention (or specific embodiments thereof) can be achieved by providing a recording sheet which comprises a paper substrate and a material selected from the group consisting of monomeric amino acids, monomeric hydroxy acids, monomeric polycarboxyl compounds, and mixtures thereof. Another embodiment of the present invention is directed to a recording sheet which comprises a substrate and a material selected from the group consisting of monomeric amino acids, monomeric hydroxy acids, and mixtures thereof.

## 55 DETAILED DESCRIPTION OF THE INVENTION

The recording sheets of the present invention comprise a substrate and at least one compound selected from the group consisting of amino acids, hydroxy acids, polycarboxyl compounds, and mixtures thereof. Any suitable substrate can be employed. Examples include transparent materials, such as polyester, including Mylar™, available from E.I. Du Pont de Nemours & Company, Melinex™, available from Imperial Chemicals, Inc., Celanar™, available from Celanese Corporation, polyethylene naphthalates, such as Kaladex PEN Films, available from Imperial Chemicals, Inc., polycarbonates such as Lexan™, available from General Electric

Company, polysulfones, such as those available from Union Carbide Corporation, polyether sulfones, such as those prepared from 4,4'-diphenyl ether, such as Udel™, available from Union Carbide Corporation, those prepared from disulfonyl chloride, such as Victrex™, available from ICI America Incorporated, those prepared from biphenylene, such as Astrel™, available from 3M Company, poly(arylene sulfones), such as those prepared from crosslinked poly(arylene ether ketone sulfones), cellulose triacetate, polyvinylchloride cellophane, polyvinyl fluoride, polyimides, and the like, with polyester such as Mylar™ being preferred in view of its availability and relatively low cost. The substrate can also be opaque, including opaque plastics, such as Teslin™, available from PPG Industries, and filled polymers, such as Melinex®, available from ICI. Filled plastics can also be employed as the substrate, particularly when it is desired to make a "never-tear paper" recording sheet. Paper is also suitable, including plain papers such as Xerox® 4024, diazo papers, or the like.

In one embodiment of the present invention, the substrate comprises sized blends of hardwood kraft and softwood kraft fibers containing from about 10 to 90 percent by weight soft wood and from about 10 to about 90 percent by weight hardwood. Examples of hardwood include Seagull W dry bleached hardwood kraft, present in one embodiment in an amount of about 70 percent by weight. Examples of softwood include La Tuque dry bleached softwood kraft, present in one embodiment in an amount of about 30 percent by weight. These substrates can also contain fillers and pigments in any effective amounts, typically from about 1 to about 60 percent by weight, such as clay (available from Georgia Kaolin Company, Astro-fil 90 clay, Engelhard Ansilex clay), titanium dioxide (available from Tioxide Company—Anatase grade AHR), calcium silicate CH-427-97-8, XP-974 (J.M. Huber Corporation), and the like. The sized substrates can also contain sizing chemicals in any effective amount, typically from about 0.25 percent to about 25 percent by weight of pulp, such as acidic sizing, including Mon size (available from Monsanto Company), alkaline sizing such as Hercon-76 (available from Hercules Company), Alum (available from Allied Chemicals as Iron free alum), retention aid (available from Allied Colloids as Percol 292), and the like. The preferred internal sizing degree of papers selected for the present invention, including commercially available papers, varies from about 0.4 to about 5,000 seconds, and papers in the sizing range of from about 0.4 to about 300 seconds are more preferred, primarily to decrease costs. Preferably, the selected substrate is porous, and the porosity value of the selected substrate preferably varies from about 100 to about 1,260 milliliters per minute and preferably from about 50 to about 600 milliliters per minute to enhance the effectiveness of the recording sheet in ink jet processes. Preferred basis weights for the substrate are from about 40 to about 400 grams per square meter, although the basis weight can be outside of this range.

Illustrative examples of commercially available internally and externally (surface) sized substrates suitable for the present invention include Diazo papers, offset papers, such as Great Lakes offset, recycled papers, such as Conservatree, office papers, such as Automimeo, Eddy liquid toner paper and copy papers available from companies such as Nekoosa, Champion, Wiggins Teape, Kymmene, Modo, Domtar, Veitsiluoto and Sanyo, and the like, with Xerox® 4024™ papers and sized calcium silicate-clay filled papers being particularly preferred in view of their availability, reliability, and low print through. Pigmented filled plastics, such as

Teslin (available from PPG industries), are also preferred as supporting substrates.

The substrate can be of any effective thickness. Typical thicknesses for the substrate are from about 50 to about 500 microns, and preferably from about 100 to about 125 microns, although the thickness can be outside these ranges.

Situated on the substrate of the present invention is a material selected from the group consisting of amino acids, hydroxy acids, polycarboxyl compounds, and mixtures thereof.

Amino acids generally are those compounds having both an amine functional group and an acid functional group. Examples of suitable amino acids include (I) those of the general formula  $R_1-(CH_2)_n-CH_2-(NHR_3)-COOH$ , wherein  $R_1$  is selected from the group consisting of alkyl, phenyl, hydroxyl, mercaptyl, sulfonic acid, alkyl sulfonic acid, alkyl mercaptyl, phenol, thio, carboxyl, indole, acetamide alkane, 1-alkyl indole, imidazole, aminophenyl, carboxy alkyl, amido alkyl, glutamyl, amino carbonyl, alkyl thio alkyl, amino alkyl, dihydroxy phenyl, vinyl, allyl, amino sulfamoyl, guanidyl alkane, benzyloxy phenyl, S-carbamyl, dicarboxy alkyl, carbobenzyloxy amine, S-trityl, tert-alkoxy carbonyl amine, S-tert alkylthio, S-carboxyalkyl, alkyl sulfoxide alkane, alkyl sulfoximine, hydroxy alkyl, mercaptyl alkyl, thiazolyl, aminoalkane, and amine,  $R_2$  is hydrogen,  $R_3$  is selected from the group consisting of hydrogen, carbobenzyloxy, glycyl, N-tert-butoxy carbonyl, and acetyl, and  $n$  represents the number of repeating units, such as (a) when  $R_1=CH_3$ ,  $R_2=H$ ,  $R_3=H$ , and  $n$  varies from 0 to 5, including (1)  $n=0$ , alanine  $CH_3CH(NH_2)COOH$  (Aldrich 13,522-4, 16,265-5, A2, 680-2); (2)  $n=1$ , 2-aminobutyric acid  $CH_3(CH_2)CH(NH_2)COOH$  (Aldrich 16,266-3, 11,612-2, 23,438-9); (3)  $n=2$ , norvaline  $CH_3(CH_2)_2CH(NH_2)COOH$  (Aldrich 22,284-4); (4)  $n=3$ , 35 norleucine  $CH_3(CH_2)_3CH(NH_2)COOH$  (Aldrich 17,109-3); (5)  $n=5$ , 2-amino caprylic acid  $CH_3(CH_2)_5CH(NH_2)COOH$  (Aldrich 21,770-0); (b) when  $R_1=C_6H_5$ ,  $R_2=H$ ,  $R_3=H$ , and  $n$  varies from 0 to 5, including (1)  $n=0$ , 2-phenyl glycine  $C_6H_5CH(NH_2)COOH$  (Aldrich P2, 550-7); (2)  $n=1$ , phenyl alanine  $C_6H_5CH_2CH(NH_2)COOH$  (Aldrich 14,796-6, P1,700-8); (3)  $n=2$ , homophenyl alanine  $C_6H_5(CH_2)_2CH(NH_2)COOH$  (Aldrich 29,435-7, 29,436-5, 29,437-3); (c) when  $n=1$ ,  $R_2=H$ ,  $R_3=H$ , and  $R_1$  varies, including (1)  $R_1=HO$ , such as serine  $HOCH_2CH(NH_2)COOH$  (Aldrich S259-7); (2)  $R_1=HS$ , such as cysteine  $HSCH_2CH(NH_2)COOH$  (Aldrich 86,167-7, 16,814-9); (3)  $R_1=HO_3S$ , such as cysteic acid monohydrate  $HO_3SCH_2CH(NH_2)COOH-H_2O$  (Aldrich 85,189-2); (4)  $R_1=HO_3SCH_2$ , such as homocysteic acid  $HO_3SCH_2CH_2CH(NH_2)COOH$  (Aldrich 21,974-6); (5)  $R_1=(CH_3)_2SH$ , such as leucine  $(CH_3)_2CHCH_2CH(NH_2)COOH$  (Aldrich 16,272-8); (6)  $R_1=HOC_6H_4$ , such as tyrosine  $4-HOC_6H_4CH_2CH(NH_2)COOH$  (Aldrich 85,545-6, 14,572-6, T9,040-9); (7)  $R_1=S$ , such as cystine  $[S-CH_2CH(NH_2)COOH]_2$  (Aldrich C12,200-9, 28,546-3, 29,867-0); (8)  $R_1=HOOC$ , such as aspartic acid  $HOOCCH_2CH(NH_2)COOH$  (Aldrich A9,309-7, 21,909-6, A9,310-0); (9)  $R_1=[C_3H_3(-O)(OH)N]$ , such as leucenol and mimosine  $C_5H_3(-O)(OH)NCH_2CH(NH_2)COOH$  (Aldrich M8,761-4); (10)  $R_1=CH_3CONH(CH_2)_3$ , such as acetyl-L-lysine  $CH_3CONH(CH_2)_3CH_2CH(NH_2)COOH$  (Aldrich 11,579-7); (11)  $R_1=C_6H_5NH$ , such as tryptophan  $C_8H_7NHCH_2CH(NH_2)COOH$  (Aldrich 15,628-0, 16,269-8, T9,020-4); (12)  $R_1=(C_6H_5)_3CS$ , such as (S)-trityl-L-cysteine  $(C_6H_5)_3SCCH_2CH(NH_2)COOH$  (Aldrich 16,473-9); (13)  $R_1=C_8H_6N(CH_3)$ , such as 1-methyl D,L-tryptophan

$C_8H_6N(CH_3)CH_2CH(NH_2)COOH$  (Aldrich 86,064-6); (14)  $R_1=C_3H_3N_2$ , such as histidine  $C_3H_3N_2CH_2CH(NH_2)COOH$  (Aldrich 15,168-8, 21,973-8); (15)  $R_1=H_2NC_6H_4$ , such as 4-amino phenylalanine hydrate  $H_2NC_6H_4CH_2CH(NH_2)COOH \cdot xH_2O$  (Aldrich 85,870-6, 34,824-4, 34,825-2); (16)  $R_1=HOOCCH_2$ , such as glutamic acid  $HOOCCH_2CH_2CH(NH_2)COOH$  (Aldrich 12,843-0, 85,735-1 and G279-6); (17)  $R_1=H_2NCOCH_2$ , such as glutamine  $H_2NCOCH_2CH_2CH(NH_2)COOH$  (Aldrich G,320-2); (18)  $R_1=HOOCCH_2CH_2CH(COOH)NHCOCH_2$ , such as Y-L-glutamyl-L-glutamic acid  $HOOCCH_2CH_2CH(COOH)NHCOCH_2CH_2CH(NH_2)COOH$  (Aldrich 85,927-3); (19)  $R_1=C_6H_5CH_2CH(COOH)NHCOCH_2$ , such as N-(y-L-glutamyl) phenylalanine  $C_6H_5CH_2CH(COOH)NHCOCH_2CH_2CH(NH_2)COOH$  (Aldrich 86,020-4); (20)  $R_1=H_2NCO$ , such as asparagine  $H_2NCOCH_2CH(NH_2)COOH$  (Aldrich A9,300-3, 21,911-8, 15,357-5, 17,653-2); (21)  $R_1=H_2NCONH(CH_2)_2$ , such as citrulline  $H_2NCONH(CH_2)_2CH(NH_2)COOH$  (Aldrich 85,572-3, C<sub>8</sub>,370-8); (22)  $R_1=C_2H_5SCH_2$ , such as ethionine  $C_2H_5SCH_2CH_2CH(NH_2)COOH$  (Aldrich 21,932-0, 10,040, 21,929-9); (23)  $R_1=H_2N(CH_2)_3$ , such as lysine  $H_2N(CH_2)_4CH(NH_2)COOH$  (Aldrich 27,414-3, 16,971-4) and lysine hydrate  $H_2N(CH_2)_4CH(NH_2)COOH \cdot H_2O$  (Aldrich 28,170-0, 28,267-7); (24)  $R_1=(HO)_2C_6H_3$ , such as DOPA [3-(3,4-dihydroxy phenyl)-alanine]  $(HO)_2C_6H_3CH_2CH(NH_2)COOH$  (Aldrich 10,216-4 and 15,431-8); (25)  $R_1=(H_2C=CH)_2$ , such as 2-amino-4-pentanoic acid  $H_2C=CHCH_2CH(NH_2)COOH$  (Aldrich 28,501-3, 17,344-4); (26)  $R_1=H_2NSO_2CH_2$ , such as 2-amino-4-sulfamoyl butyric acid  $H_2NSO_2CH_2CH_2CH(NH_2)COOH$  (Aldrich 31,096-4); (27)  $R_1=[H_2NC(=NH)NH(CH_2)_2]$ , such as arginine  $H_2NC(=NH)NH(CH_2)_3CH(NH_2)COOH$  (Aldrich 85,853-6, A9,240-6); (28)  $R_1=C_6H_5CH_2OC_6H_4$ , such as carbobenzyl-L-tyrosine  $C_6H_5CH_2OC_6H_4CH_2CH(NH_2)COOH$  (Aldrich 85,583-9); (29)  $R_1=H_2NCOS$ , such as S-carbamyl-L-cysteine  $H_2NCOSCH_2CH(NH_2)COOH$  (Aldrich 11,578-9); (30)  $R_1=(CH_3)_3COOCNH(CH_2)_3$ , such as N- $\epsilon$ (tert-butoxy carbonyl)-L-lysine  $(CH_3)_3COOCNH(CH_2)_3CH_2CH(NH_2)COOH$  (Aldrich 35,966-1); (31)  $R_1=(CH_3)_3CSS$ , such as S-(tert butylthio)-L-cysteine  $(CH_3)_3CSSCH_2CH(NH_2)COOH$  (Aldrich 23,235-1); (32)  $R_1=(HOOC)_2CH$ , such as L-y-carboxy glutamic acid  $(HOOC)_2CHCH_2CH(NH_2)COOH$  (Aldrich 28,408-4); (33)  $R_1=C_6H_5CH_2OOCNH(CH_2)_3$ , such as N-carbobenzoyloxy-L-lysine  $C_6H_5CH_2OOCNH(CH_2)_4CH(NH_2)COOH$  (Aldrich C<sub>800</sub>-8); (34)  $R_1=HOOCCH_2S$ , such as S-carboxymethyl-L-cysteine  $HOOCCH_2SCH_2CH(NH_2)COOH$  (Aldrich 85,121-3); (35)  $R_1=CH_3SCH_2$ , such as methionine  $CH_3S(CH_2)_2CH(NH_2)COOH$  (Aldrich M885-1, 85,590-1, and 15,169-6), (36)  $R_1=CH_3SOCH_2$ , such as methionine sulfoxide  $CH_3SO(CH_2)_2CH(NH_2)COOH$  (Aldrich 85,126-4); (37)  $R_1=CH_3S(O)(=NH)CH_2$ , such as L-methionine sulfoximine  $CH_3S(O)(=NH)(CH_2)_2CH(NH_2)COOH$  (Aldrich 85,589-8); (38)  $R_1=HOCH_2$  such as homoserine  $HOCH_2CH_2CH(NH_2)COOH$  (Aldrich 21,977-0); (39)  $R_1=HSCH_2$ , such as homocysteine  $HSCH_2CH_2CH(NH_2)COOH$  (Aldrich 19,314-3, 21,974-6); (40)  $R_1=C_3H_2NS$ , such as 3-(2-thiazolyl)-D,L-alanine  $C_3H_2NSCH_2CH(NH_2)COOH$  (Aldrich 86,219-3); (d) when n=1,  $R_2=H$ ,  $R_3=COCH_2NH_2$ , and  $R_1$  varies, including (1)  $R_1=(CH_3)_2CH$ , such as glycyl L-leucine  $(CH_3)_2CHCH_2CH(NHCOCH_2NH_2)COOH$  (Aldrich 85,007-1); (2)  $R_1=4(HO)C_6H_4$ , such as glycyl L-tyrosine dihydrate

4(HO)C<sub>6</sub>H<sub>4</sub>CH<sub>2</sub>CH(NHCOCH<sub>2</sub>NH<sub>2</sub>)COOH.2H<sub>2</sub>O (Aldrich 85,872-2); (3)  $R_1=HOOCCH_2$ , such as glycyl-L-glutamic acid  $HOOCCH_2CH_2CH(NHCOCH_2NH_2)COOH$  (Aldrich 85,160-4); (e) when n=0,  $R_2=H$ ,  $R_3=H$ , and  $R_1$  varies, including (1)  $R_1=CH_3CH(OH)$ , such as threonine  $CH_3CH(OH)CH(NH_2)COOH$  (Aldrich T3,422-3); (2)  $R_1=(CH_3)_2CH$ , such as valine  $(CH_3)_2CHCH(NH_2)COOH$  (Aldrich 85,598-7, 16,267-1, V70-5); (3)  $R_1=C_2H_5CH(CH_3)$ , such as isoleucine  $C_2H_5CH(CH_3)CH(NH_2)COOH$  (Aldrich 15,171-8, 29,868-9, 29,865-4); (4)  $R_1=HOC_6H_4$ , such as D-4-hydroxy phenyl glycine  $HOC_6H_4CH(NH_2)COOH$  (Aldrich 21,533-3); (5)  $R_1=C_2H_5CH(OH)$ , such as 3-hydroxynorvaline  $C_2H_5CH(OH)CH(NH_2)COOH$  (Aldrich 28,617-6); (f) when n=1,  $R_2=H$ ,  $R_3=COCH_3$ , and  $R_1$  varies, including (1)  $R_1=HOOCCH_2$ , such as N-acetyl-L-glutamic acid  $HOOCCH_2CH_2CH(NHCOCH_3)COOH$  (Aldrich 85,564-20); (2)  $R_1=CH_3SCH_2$ , such as N-acetyl-methionine  $CH_3SCH_2CH_2CH(NHCOCH_3)COOH$  (Aldrich A1,790-0, 85,554-5); (3)  $R_1=C_3H_3N_2$ , such as N- $\alpha$ -acetyl-L-histidine monohydrate  $C_3H_3N_2CH_2CH(NHCOCH_3)COOH \cdot H_2O$  (Aldrich 85,754-8); (4)  $R_1=C_6H_6NH$ , such as N-acetyl tryptophan  $C_8H_6NHCH_2CH(NHCOCH_3)COOH$  (Aldrich 85,580-4); (5)  $R_1=HS$ , such as N-acetyl-L-cysteine  $HSCH_2CH(NHCOCH_3)COOH$  (Aldrich 13,806-1); (6)  $R_1=C_6H_5$ , such as N-acetyl-L-phenylalanine  $C_6H_5CH_2CH(NHCOCH_3)COOH$  (Aldrich 85,745-9); (7) N-acetyl-D,L-penicillamine  $(CH_3)_2C(SH)CH(NHCOCH_3)COOH$  (Aldrich A1,900-8); (g) when n=0,  $R_2=CH_3$ ,  $R_3=H$ , and  $R_1$  varies, including (1)  $R_1=(CH_3)_2CH$ , such as 2-aminobutyric acid  $(CH_3)_2C(CH_3)(NH_2)COOH$  (Aldrich 85,099-3); (2)  $R_1=4(HO)C_6H_4CH_2$ , such as D,L- $\alpha$ -methyl tyrosine  $4(HO)C_6H_4CH_2C(CH_3)(NH_2)COOH$  (Aldrich 12,069-3); (3)  $R_1=(HO)_2C_6H_3CH_2$ , such as (-)-3-(3,4-dihydroxyphenyl)-2-methyl-L-alanine sesquihydrate  $(HO)_2C_6H_3CH_2C(CH_3)(NH_2)COOH \cdot 1.5H_2O$  (Aldrich 85,741-6); (4)  $R_1=C_6H_5CH_2$ , such as  $\alpha$ -methyl-D,L-phenylalanine  $C_6H_5CH_2C(CH_3)(NH_2)COOH$  (Aldrich 28,665-6); (h) when n=1,  $R_2=H$ ,  $R_3=[COCH(NH_2)CH_3]$ , and  $R_1$  varies, including (1)  $R_1=C_2H_5$ , such as D,L-alanyl-DL-norvaline  $C_2H_5SCH_2CH[NHCOCH(NH_2)CH_3]COOH$  (Aldrich 85,001-2); (2)  $R_1=C_6H_5$ , such as D,L-alanyl-D,L-phenylalanine  $C_6H_5CH_2CH[NHCOCH(NH_2)CH_3]COOH$  (Aldrich 85,002-0); (i) when n=0,  $R_2=H$ ,  $R_3=[COOC(CH_3)_3]$ , and  $R_1$  varies, including (1)  $R_1=C_2H_5CH(CH_3)$ , such as N-(tert-butoxy carbonyl)-L-isoleucine  $C_2H_5CH(CH_3)CH[NHCOOC(CH_3)_3]COOH$  (Aldrich 35,965-3); (2)  $R_1=H_2N(CH_2)_4$ , such as N- $\alpha$ -(tert-butoxy carbonyl)-L-lysine  $H_2N(CH_2)_4CH[NHCOOC(CH_3)_3]COOH$  (Aldrich 35,968-8); (3)  $R_1=C_6H_5CH_2$ , such as N-(tert-butoxy carbonyl)-L-phenylalanine  $C_6H_5CH_2CH[NHCOOC(CH_3)_3]COOH$  (Aldrich 13,456-2); (4)  $R_1=HOCH_2$ , such as N-(tert-butoxy carbonyl)-L-serine  $HOCH_2CH[NHCOOC(CH_3)_3]COOH$  (Aldrich 35,969-6); (5)  $R_1=CH_3CH(OH)$ , such as N-(tert-butoxy carbonyl)-L-threonine  $CH_3CH(OH)CH[NHCOOC(CH_3)_3]COOH$  (Aldrich 35,971-8); (6)  $R_1=(CH_3)_2CH$ , such as N-(tert-butoxy carbonyl)-L-valine  $(CH_3)_2CHCH[NHCOOC(CH_3)_3]COOH$  (Aldrich 35,972-6); (j) when n=0,  $R_2=H$ ,  $R_3=[COOCH_2C_6H_5]$ , and  $R_1$  varies, including (1)  $R_1=CH_3$ , such as carbobenzoyloxy-alanine  $CH_3CH[NHCOOCH_2C_6H_5]COOH$  (Aldrich 85,069-1, 15,689-2); (2)  $R_1=H_2NC(=NH)NH(CH_2)_3$ , such as N-carbobenzoyloxy-L-arginine  $H_2N(=NH)NH(CH_2)_3CH[NHCOOCH_2C_6H_5]COOH$  (Aldrich 16,263-9); (3)  $R_1=H_2NCOCH_2$ , such as carbobenzoyloxy-L-asparagine  $H_2NCOCH_2CH[NHCOOCH_2C_6H_5]COOH$  (Aldrich C<sub>640</sub>-

4); (4)  $R_1=HOOCCH_2$ , such as N-carbobenzyloxy-L-aspartic acid  $HOOCCH_2CH[NHCOOCH_2C_6H_5]COOH$  (Aldrich 16,262-0); (5)  $R_1=H_2NCOCH_2CH_2$ , such as carbobenzyloxy-L-glutamine  $H_2NCOCH_2CH_2CH[NHCOOCH_2C_6H_5]COOH$  (Aldrich 16,264-7); (6)  $R_1=H_2N(CH_2)_4$ , such as N-(carbobenzyloxy)-L-lysine  $H_2N(CH_2)_4CH[NHCOOCH_2C_6H_5]COOH$  (Aldrich 35,979-3); (7)  $R_1=C_6H_5CH_2$ , such as N-(carbobenzyloxy)-L-phenylalanine  $C_6H_5CH_2CH[NHCOOCH_2C_6H_5]COOH$  (Aldrich 35,980-7); (8)  $R_1=HOCH_2$ , such as carbobenzyloxy-serine  $HOCH_2CH[NHCOOCH_2C_6H_5]COOH$  (Aldrich 86,070, C<sub>900</sub>-4); (9)  $R_1=(CH_3)_2CH$ , such as carbobenzyloxy-L-valine  $(CH_3)_2CHCH[NHCOOCH_2C_6H_5]COOH$  (Aldrich 29,352-0); and the like.

Also suitable are (II) amino acids of the general formula  $R_1-(CH_2)_n-CH_2-(NHR_2)-COOH.XH$ , wherein  $R_1$  is selected from the group consisting of amine, amino alkane, guanidyl alkane, and phenyl alkyl,  $R_2$  is hydrogen or alkyl, and  $X$  is an anion, such as  $Cl^-$ ,  $Br^-$ ,  $I^-$ ,  $SO_3^-$ , or the like, such as (a) when  $n=1$ ,  $R_2=H$ ,  $R_3=H$ , and  $R_1$  varies, including (1)  $R_1=H_2N$ , such as 2,3-diamino propionic acid monohydrochloride  $H_2NCH_2CH(NH_2)COOH.HCl$  (Aldrich 21,963-0); (2)  $R_1=H_2N$ , such as 2,3-diamino propionic acid monohydrobromide  $H_2NCH_2CH(NH_2)COOH.HBr$  (Aldrich D2,400-5); (3) when  $R_1=H_2N(CH_2)_2$ , such as ornithine hydrochloride  $H_2N(CH_2)_3CH(NH_2)COOH.HCl$  (Aldrich 22,285-2, Aldrich 0-830-5); (4)  $R_1=[H_2NC(=NH)NH(CH_2)_3]$ , such as homoarginine hydrochloride  $H_2NC(=NH)NH(CH_2)_3CH_2CH(NH_2)COOH.HCl$  (Aldrich 15,711-2); (5)  $R_1=[H_2NC(=NH)NH(CH_2)_2]$ , such as arginine hydrochloride  $H_2NC(=NH)NH(CH_2)_3CH(NH_2)COOH.HCl$  (Aldrich A9,260-0); (6)  $R_1=H_2NCH_2$ , such as 2,4-diaminobutyric acid dihydrochloride  $H_2NCH_2CH_2CH(NH_2)COOH.2HCl$  (Aldrich 23,776-0, 85,019-5); (7)  $R_1=H_2N(CH_2)_3$ , such as lysine monohydrochloride  $H_2N(CH_2)_4CH(NH_2)COOH.HCl$  (Aldrich L460-5, 26,068-1,28,171-9) and lysine dihydrochloride  $H_2N(CH_2)_4CH(NH_2)COOH.2HCl$  (Aldrich 36,022-8); (8) when  $R_1=C_6H_5CH(CH_3)$  and  $n=0$ , such as  $\beta$ -methyl-D,L-phenylalanine hydrochloride  $C_6H_5CH(CH_3)CH(NH_2)COOH.HCl$  (Aldrich 21,703-4); (9) when  $R_1=H_2N(CH_2)_2$  and  $R_2=CH_3$ , such as 2-methylornithine hydrochloride monohydrate  $H_2N(CH_2)_3C(CH_3)(NH_2)COOH.HClH_{20}$  (Aldrich 28,409-2); and the like.

Also suitable are (III) amino acids of the general formula  $H_2N-R-COOH$  and their salts, wherein  $R$  is selected from the group consisting of alkane, phenyl, benzyl, alkyl phenyl, phenyl dialkoxy, alkyl cycloalkane, phenol, aminophenyl, diamino phenyl, glycyl, amino benzoyl alkane, amino cycloalkane, methoxy, amino benzophenone, imino phenyl, acetyl alkane, phenyl alkene, phenyl amido alkane, hydroxy alkyl phenyl, dialkyl hydroxy alkyl amino alkane, and benzyl carbonyl, such as (a) when  $R=(CH_2)_n$  and  $n$  varies from 1 to 12, including (1) [ $n=1$ ], glycine  $H_2NCH_2COOH$  (Aldrich G620-1) and glycine hydrochloride  $H_2NCH_2COOH.HCl$  (Aldrich 21,950-9); (2) [ $n=2$ ],  $\beta$ -alanine  $H_2N(CH_2)_2COOH$  (Aldrich 23,972-0); (3) [ $n=3$ ], 4-aminobutyric acid  $H_2N(CH_2)_3COOH$  (Aldrich A4,440-1); (4) [ $n=4$ ], 5-aminovaleric acid  $H_2N(CH_2)_4COOH$  (Aldrich 12,318-8) and 5-aminovaleric acid hydrochloride  $H_2N(CH_2)_4COOH.HCl$  (Aldrich 19,433-6); (5) [ $n=5$ ], 6-amino caproic acid  $H_2N(CH_2)_5COOH$  (Aldrich A4,460-6); (6) [ $n=6$ ], 7-aminoheptanoic acid  $H_2N(CH_2)_6COOH$  (Aldrich 28,463-7); (7) [ $n=7$ ], 8-amino caprylic acid  $H_2N(CH_2)_7COOH$  (Aldrich 85,529-4); (8) [ $n=10$ ], 11-amino undecanoic acid  $H_2N(CH_2)_{10}COOH$  (Aldrich A8260-5); (9)

[ $n=11$ ], 12-amino dodecanoic acid  $H_2N(CH_2)_{11}COOH$  (Aldrich 15,924-7); (b) when  $R$  is different in each case, including (1)  $R=C_6H_4$ , such as amino benzoic acid  $H_2NC_6H_4COOH$  (Aldrich 10,053-6 and 12,767-1) and 3-amino benzoic acid hydrochloride  $H_2NC_6H_4COOH.HCl$  (Aldrich 28,965-5); (2)  $R=C_6H_4CH_2$ , such as 4-amino phenyl acetic acid  $H_2NC_6H_4CH_2COOH$  (Aldrich A7,135-2); (3)  $R=CH_2C_6H_4$ , such as 4-amino methyl benzoic acid  $H_2NCH_2C_6H_4COOH$  (Aldrich 28,374-6); (4)  $R=C_6H_3(CH_3)$ , such as 5-amino-2-methyl benzoic acid  $H_2NC_6H_3(CH_3)COOH$  (Aldrich A6,300-7, A6, 280-9, A6220-0); (5)  $R=C_6H_2(OCH_3)_2$ , such as 2-amino-4,5-dimethoxy benzoic acid  $H_2NC_6H_2(OCH_3)_2COOH$  (Aldrich 25,204-2); (6)  $R=CH_2C_6H_{10}$ , such as 4-amino methyl cyclohexane carboxylic acid  $H_2NCH_2C_6H_{10}COOH$  (Aldrich 85,765-3); (7)  $R=C_6H_3-2(OH)$ , such as 5-amino salicylic acid  $H_2NC_6H_3-2(OH)COOH$  (Aldrich A7,980-9); (8)  $R=H_2NC_6H_3$ , such as 3,5-diaminobenzoic acid  $(H_2N)_2C_6H_3COOH$  (Aldrich D 1280-5); (9)  $R=C_6H_4CONHCH_2$ , such as 4-aminohippuric acid  $H_2NC_6H_4CONHCH_2COOH$  (Aldrich 12,295-5); (10)  $R=CH_2CONHCH_2$ , such as glycyl glycine  $H_2NCH_2CONHCH_2COOH$  (Aldrich G780-1); (11)  $R=CH_2(CONHCH_2)_2$ , such as glycyl glycyl glycine  $H_2NCH_2(CONHCH_2)_2COOH$  (Aldrich 86,008-5); (12)  $R=[C_6H_4CONHCH_2CH_2]$ , such as N-(4-aminobenzoyl)- $\beta$ -alanine  $H_2NC_6H_4CONHCH_2CH_2COOH$  (Aldrich 23,347-1); (13)  $R=C_6H_4CONH(CH_2)_5$ , such as N-(4-aminobenzoyl)-6-aminocaproic acid  $H_2NC_6H_4CONH(CH_2)_2COOH$  (Aldrich 23,349-8); (14)  $R=C_6H_3-1,3-(COOH)$ , such as 5-amino isophthalic acid  $H_2NC_6H_3-1,3-(COOH)_2$  (Aldrich 18,627-9); (15)  $R=C_5H_8$ , such as 1-amino-1-cyclopentane carboxylic acid  $H_2NC_5H_8COOH$  (Aldrich A4,810-5); (16)  $R=C_3H_4$ , such as 1-amino-1-cyclopropane carboxylic acid hemihydrate  $H_2NC_3H_4COOH.1/2H_2O$  (Aldrich 28,872-0) and 1-amino-1-cyclopropane carboxylic acid hydrochloride  $H_2NC_3H_4COOH.HCl$  (Aldrich 30,408-5); (17)  $R=C_6H_4CH=CH$ , such as 4-amino cinnamic acid hydrochloride  $H_2NC_6H_4CH=CHCOOH.HCl$  (Aldrich A4,710-9); (18)  $R=COCH_2CH_2$ , such as succinamic acid  $H_2NCOCH_2CH_2COOH$  (Aldrich 13,437-6); (19)  $R=OCH_2$ , such as carboxymethoxylamine hemihydrate  $(H_2NOCH_2COOH)_2HCl$  (Aldrich C<sub>1,340</sub>-8); (20)  $R=NHC_6H_4$ , such as 2-hydrazino benzoic acid hydrochloride  $H_2NNHC_6H_4COOH.HCl$  (Aldrich 32,430-2); (21)  $R=CONH(NH_2)CONHCH_2$ , such as allantoic acid (diureidoacetic acid)  $(H_2NCONH_2)CHCOOH$  (Aldrich 21,784-0); (22)  $R=C_6H_4COC_6H_4NH_2$ , such as 2-aminobenzophenone-2-carboxylic acid  $H_2NC_6H_4COC_6H_4NH_2COOH$  (Aldrich 15,327-3); (23)  $R=C(=NH)N(CH_3)CH_2$ , such as creatine monohydrate  $H_2NC(=NH)N(CH_3)CH_2COOH.H_2O$  (Aldrich 85,524-3, 29,119-6); and the like.

Also suitable are (IV) imino acids containing NH and COOH groups, such as (1) n-trityl glycine  $[(C_6H_5)_3CNHCH_2COOH]$  (Aldrich 30,151-5); (2) 2-acetamido acrylic acid  $H_2C=C(NHCOCH_3)COOH$  (Aldrich A140-1); (3) 4-acetamido benzoic acid  $CH_3CONHC_6H_4COOH$  (Aldrich 13,333-7); (4)  $\alpha$ -acetamido cinnamic acid  $C_6H_5CH=C(NHCOCH_3)COOH$  (Aldrich 21,385-3); (5) 6-acetamido hexanoic acid  $CH_3CONH(CH_2)_2COOH$  (Aldrich 19,430-1); (6) acetamido acetic acid  $CH_3CONHCH_2COOH$  (Aldrich A1,630-0); (7) N-(2-mercaptopropionyl) glycine  $CH_3CH(SH)CONHCH_2COOH$  (Aldrich 28,096-8); and the like.

Also suitable are (V) amino acids of the general formula  $H_2N-(R)-SO_3H$ , wherein  $R$  is selected from the group con-

sisting of alkane, alkylene oxide, phenyl, naphthyl, amino benzene, and acetamido alkane, such as (a) when R=(CH<sub>2</sub>)<sub>n</sub> and n varies from 1 to 12, including (1) n=0, such as sulfamic acid H<sub>2</sub>NSO<sub>3</sub>H (Aldrich 24,278-0); (2) (n=1), R=CH<sub>2</sub>, such as amino methane sulfonic acid H<sub>2</sub>N(CH<sub>2</sub>)SO<sub>3</sub>H (Aldrich 12,744-2); (3) (n=2), R=(CH<sub>2</sub>)<sub>2</sub>, such as  $\alpha$ -2-aminoethane sulfonic acid H<sub>2</sub>N(CH<sub>2</sub>)<sub>2</sub>SO<sub>3</sub>H (Aldrich 15,224-2); (4) (n=3), R=(CH<sub>2</sub>)<sub>3</sub>, such as 3-amino-1-propane sulfonic acid H<sub>2</sub>N(CH<sub>2</sub>)<sub>3</sub>SO<sub>3</sub>H (Aldrich A7,610-9); (b) when R is different from (CH<sub>2</sub>)<sub>n</sub>, including (1) R=CH<sub>2</sub>CH<sub>2</sub>O, such as 2-amino ethyl hydrogen sulfate H<sub>2</sub>NCH<sub>2</sub>CH<sub>2</sub>OSO<sub>3</sub>H (Aldrich A5,440-7); (2) R=C<sub>6</sub>H<sub>4</sub>, such as sulfanilic acid H<sub>2</sub>NC<sub>6</sub>H<sub>4</sub>SO<sub>3</sub>H (Aldrich 11,273-9); (3) R=C<sub>10</sub>H<sub>6</sub>, such as 2-amino-1-naphthalene sulfonic acid H<sub>2</sub>NC<sub>10</sub>H<sub>6</sub>SO<sub>3</sub>H (Aldrich 29,113-7); (4) R=H<sub>2</sub>NC<sub>6</sub>H<sub>3</sub>, such as 2,5-diamino benzene sulfonic acid (H<sub>2</sub>N)<sub>2</sub>C<sub>6</sub>H<sub>3</sub>SO<sub>3</sub>H (Aldrich 15,350-8); (5) R=COCH<sub>2</sub>NHCH<sub>2</sub>CH<sub>2</sub>, such as [N-(2-acetamido) 2-amino ethane sulfonic acid] H<sub>2</sub>NCOCH<sub>2</sub>NHCH<sub>2</sub>CH<sub>2</sub>SO<sub>3</sub>H (Aldrich 85,760-2); and the like.

Also suitable are (VI) amino acids of the general formula NH<sub>2</sub>(R)P(O)(OH)<sub>2</sub>, wherein R is selected from the group consisting of alkylene oxide, alkane, and phenyl, including (1) when R=CH<sub>2</sub>CH<sub>2</sub>O, such as 2-amino ethyl dihydrogen phosphate H<sub>2</sub>NCH<sub>2</sub>CH<sub>2</sub>OP(O)(OH)<sub>2</sub> (Aldrich 29,286-9); (2) when R=CH<sub>2</sub>CH<sub>2</sub>, such as 2-aminoethyl phosphonic acid H<sub>2</sub>NCH<sub>2</sub>CH<sub>2</sub>P(O)(OH)<sub>2</sub> (Aldrich 26,867-4); (3) when R=(CH<sub>2</sub>)<sub>3</sub>, such as 3-aminopropyl phosphonic acid (H<sub>2</sub>N(CH<sub>2</sub>)<sub>3</sub>P(O)(OH)<sub>2</sub> (Aldrich 26,861-5); (4) when R=C<sub>6</sub>H<sub>4</sub>, such as 4-amino phenyl phosphonic acid H<sub>2</sub>NC<sub>6</sub>H<sub>4</sub>P(O)(OH)<sub>2</sub> (Aldrich 29,094-7); and the like.

Hydroxy acids generally are compounds having both a hydroxy functional group and an acid functional group. Examples of suitable hydroxy acids include (I) those of the general formula HO[R]XH, wherein R is selected from the group consisting of alkane, cycloalkane, phenyl, alkoxy phenyl, dialkoxy phenyl, alkyl phenyl, and phenyl alkene and X is an anion, such as COO<sup>-</sup>, SO<sub>3</sub><sup>-</sup>, NO<sub>3</sub><sup>-</sup>, or the like, including (1) glycolic acid HOCH<sub>2</sub>COOH (Aldrich 12473-7); (2) 10-hydroxydecanoic acid HO(CH<sub>2</sub>)<sub>9</sub>COOH (Aldrich 28,421-1); (3) 12-hydroxydodecanoic acid HO(CH<sub>2</sub>)<sub>11</sub>COOH (Aldrich 19,878-1); (4) 16-hydroxy hexadecanoic acid HO(CH<sub>2</sub>)<sub>15</sub>COOH (Aldrich 17,749-0); (5) 1-hydroxy-1-cyclopropane carboxylic acid HOC<sub>3</sub>H<sub>4</sub>COOH (Aldrich 29,388-1); (6) hydroxy benzoic acid HOC<sub>6</sub>H<sub>4</sub>COOH (Aldrich H<sub>2,000</sub>-8, 24,014-1, H<sub>2,005</sub>-9); (7) 3-hydroxy-4-methoxy benzoic acid HOC<sub>6</sub>H<sub>3</sub>(OCH<sub>3</sub>)COOH (Aldrich 22,010-8); (8) 4-hydroxy-3-methoxy benzoic acid HOC<sub>6</sub>H<sub>3</sub>(OCH<sub>3</sub>)COOH (Aldrich H<sub>3,600</sub>-1); (9) 4-hydroxy-3,5-dimethoxy benzoic acid 4-(HO)C<sub>6</sub>H<sub>2</sub>-3,5-(OCH<sub>3</sub>)<sub>2</sub>COOH (Aldrich S800-5); (10) 3-hydroxy-4,5-dimethoxy benzoic acid HOC<sub>6</sub>H<sub>2</sub>(OCH<sub>3</sub>)<sub>2</sub>COOH (Aldrich 26,845-3); (11) 2-hydroxy-3-isopropyl-6-methyl benzoic acid HOC<sub>6</sub>H<sub>2</sub>[CH(CH<sub>3</sub>)<sub>2</sub>](CH<sub>3</sub>)COOH (Aldrich 33,991-1); (12) 2-hydroxy-6-isopropyl-3-methyl benzoic acid HOC<sub>6</sub>H<sub>2</sub>[CH(CH<sub>3</sub>)<sub>2</sub>](CH<sub>3</sub>)COOH (Aldrich 34,097-9); (13) hydroxy cinnamic acid HOC<sub>6</sub>H<sub>4</sub>CH=CHCOOH (Aldrich H<sub>2,280</sub>-9, H<sub>2,300</sub>-7, H<sub>2,320</sub>-1); (14) 3-hydroxy-4-methoxy cinnamic acid HOC<sub>6</sub>H<sub>3</sub>(OCH<sub>3</sub>)CH=CHCOOH (Aldrich 10,301-2); (15) 4-hydroxy-3-methoxy cinnamic acid HOC<sub>6</sub>H<sub>3</sub>(OCH<sub>3</sub>)CH=CHCOOH (Aldrich 12,870-8); (16) 3,5-dimethoxy-4-hydroxy cinnamic acid HOC<sub>6</sub>H<sub>2</sub>(OCH<sub>3</sub>)<sub>2</sub>CH=CHCOOH (Aldrich D13,460-0); (17) 2-hydroxyhippuric acid HOC<sub>6</sub>H<sub>4</sub>CONHCH<sub>2</sub>COOH (Aldrich 13,406-6); (18) hydroxy phenyl acetic acid HOC<sub>6</sub>H<sub>4</sub>CH<sub>2</sub>COOH (Aldrich H,980-4, H<sub>4,990</sub>-1, H<sub>5,000</sub>-4);

(19) 4-hydroxy-3-methoxy phenyl acetic acid HOC<sub>6</sub>H<sub>3</sub>(OCH<sub>3</sub>)CH<sub>2</sub>COOH (Aldrich 14,364-2); (20) D,L-3-(4-hydroxyphenyl) lactic acid hydrate HOC<sub>6</sub>H<sub>4</sub>CH<sub>2</sub>CH(OH)COOH.xH<sub>2</sub>O (Aldrich 28,618-4); (21) 4-hydroxyphenyl pyruvic acid HOC<sub>6</sub>H<sub>4</sub>CH<sub>2</sub>COCOOH (Aldrich 11,428-6); (22) 4-hydroxy benzene sulfonic acid HOC<sub>6</sub>H<sub>4</sub>SO<sub>3</sub>H (Aldrich 17,150-6); (23) 3[(1,1-dimethyl-2-hydroxyethyl) amino]-2-hydroxy propane sulfonic acid HOCH<sub>2</sub>C(CH<sub>3</sub>)<sub>2</sub>NHCH<sub>2</sub>CH(OH)CH<sub>2</sub>SO<sub>3</sub>H (Aldrich 34,016-2); and the like.

Also suitable are (II) those of the general formula R<sub>1</sub>R<sub>2</sub>(OH)COOH, wherein R<sub>1</sub> and R<sub>2</sub> are each independently selected from the group consisting of alkyl, dialkyl, phenyl, alkoxy, halide, hydroxy, phenyl, dihalide vinyl acrylamide, cycloalkane, and halogenated hydroxyl phenyl, including (1) lactic acid CH<sub>3</sub>CH(OH)COOH (Aldrich L5-2); (2) 3-hydroxybutyric acid CH<sub>3</sub>CH(OH)CH<sub>2</sub>COOH (Aldrich H<sub>2,220</sub>-5); (3) 2-hydroxyisobutyric acid (CH<sub>3</sub>)<sub>2</sub>C(OH)COOH (Aldrich 32,359-4, 16,497-6); (4) 2-ethyl-2-hydroxybutyric acid (C<sub>2</sub>H<sub>5</sub>)<sub>2</sub>C(OH)COOH (Aldrich 13,843-6); (5) 2-hydroxy-3-methyl butyric acid (2-hydroxy isovaleric acid) (CH<sub>3</sub>)<sub>2</sub>CHCH(OH)COOH (Aldrich 21,983-5); (6) 2-hydroxy-2-methyl butyric acid C<sub>2</sub>H<sub>5</sub>C(CH<sub>3</sub>)(OH)COOH (Aldrich H<sub>4,000</sub>-9); (7) D,L-2-hydroxy caproic acid CH<sub>3</sub>(CH<sub>2</sub>)<sub>3</sub>CH(OH)COOH (Aldrich 21,980-0); (8) hydroxyisocaproic acid (CH<sub>3</sub>)<sub>2</sub>CHCH<sub>2</sub>CH(OH)COOH (Aldrich 21,981-9, 21,982-7); (9) D,L mandelic acid C<sub>6</sub>H<sub>5</sub>CH(OH)COOH (Aldrich M210-1); (10) (±)-4-methoxy mandelic acid CH<sub>3</sub>OC<sub>6</sub>H<sub>4</sub>CH(OH)COOH (Aldrich 29,688-0); (11) 4-bromo mandelic acid BrC<sub>6</sub>H<sub>4</sub>CH(OH)COOH (Aldrich B7,120-9); (12) D,L-3-hydroxy-4-methoxy mandelic acid HOC<sub>6</sub>H<sub>3</sub>(OCH<sub>3</sub>)CH(OH)COOH (Aldrich 23,542-3); (13) D,L-4-hydroxy-3-methoxy mandelic acid HOC<sub>6</sub>H<sub>3</sub>(OCH<sub>3</sub>)CH(OH)COOH (Aldrich 14,880-6); (14) D,L-4-hydroxy mandelic acid monohydrate HOC<sub>6</sub>H<sub>4</sub>CH(OH)COOH.H<sub>2</sub>O (Aldrich 16,832-7); (15) 3-chloro-4-hydroxy benzoic acid hemihydrate ClC<sub>6</sub>H<sub>3</sub>(OH)COOH.½H<sub>2</sub>O (Aldrich C<sub>4,460</sub>-5); (16) 2-hydroxy-3-isopropyl benzoic acid (CH<sub>3</sub>)<sub>2</sub>CHC<sub>6</sub>H<sub>3</sub>(OH)COOH (Aldrich 34,366-8); (17) 3,5-dibromohydroxy benzoic acid (Br)<sub>2</sub>C<sub>6</sub>H<sub>2</sub>(OH)COOH (Aldrich 25,134-8); (18) 3,5-dichloro hydroxy benzoic acid (Cl)<sub>2</sub>C<sub>6</sub>H<sub>2</sub>(OH)COOH (Aldrich D6,400-7); (19) benzilic acid (C<sub>6</sub>H<sub>5</sub>)<sub>2</sub>C(OH)COOH (Aldrich B519-4); (20) 2-(4-hydroxy phenoxy) propionic acid CH<sub>3</sub>CH(OCH<sub>2</sub>H<sub>4</sub>OH)COOH (Aldrich 32,899-5); (21)  $\alpha$ -hydroxy hippuric acid C<sub>6</sub>H<sub>5</sub>CONHCH(OH)COOH (Aldrich 22,387-5); (22) 3,5-diisopropyl salicylic acid [(CH<sub>3</sub>)<sub>2</sub>CH]<sub>2</sub>C<sub>6</sub>H<sub>2</sub>-2-(OH)COOH (Aldrich 13,569-0); (23) 3-chloro-4-hydroxy phenyl acetic acid ClC<sub>6</sub>H<sub>3</sub>(OH)CH<sub>2</sub>COOH (Aldrich 22,452-9); (24) D,L-12-hydroxystearic acid CH<sub>3</sub>(CH<sub>2</sub>)<sub>5</sub>CH(OH)(CH<sub>2</sub>)<sub>10</sub>COOH (Aldrich 21,996-7); (25) tropic acid C<sub>6</sub>H<sub>5</sub>CH(CH<sub>2</sub>OH)COOH (Aldrich T8,920-6); (26) 2-acrylamido glycolic acid monohydrate H<sub>2</sub>C=CHCONHCH(OH)COOH.H<sub>2</sub>O (Aldrich 26,049-5); (27) hexahydromandelic acid C<sub>6</sub>H<sub>11</sub>CH(OH)COOH (Aldrich 30,114-0, 30,115-9); and the like.

Also suitable are (III) those of the general formula (HO)<sub>2</sub>RCOOH, wherein R is selected from the group consisting of phenyl, acrylic phenyl, phenyl alkyl, phenyl hydroxy, alkyl, naphthyl, alkane amine, diphenyl alkyl, and amino alkyl, including (1) dihydroxy benzoic acid (HO)<sub>2</sub>C<sub>6</sub>H<sub>3</sub>COOH (Aldrich 12,620-9, D10,940-1, 14,935-7, D10,960-6, D10,980-0, D11,000-0); (2) 3,4-dihydroxy cinnamic acid (HO)<sub>2</sub>C<sub>6</sub>H<sub>3</sub>CH=CHCOOH (Aldrich D11,080-9); (3) 3,4-dihydroxy hydro cinnamic acid

(HO)<sub>2</sub>C<sub>6</sub>H<sub>3</sub>CH<sub>2</sub>CH<sub>2</sub>COOH (Aldrich 10,260-1); (4) D,L-3, 4-dihydroxy mandelic acid (HO)<sub>2</sub>C<sub>6</sub>H<sub>3</sub>CH(OH)COOH (Aldrich 15,161-0); (5) 3,5-dihydroxy-4-methyl benzoic acid hemihydrate CH<sub>3</sub>C<sub>6</sub>H<sub>2</sub>(OH)<sub>2</sub>COOH. $\frac{1}{2}$ H<sub>2</sub>O (Aldrich 31,848-5); (6) dihydroxy naphthoic acid (HO)<sub>2</sub>C<sub>10</sub>H<sub>5</sub>COOH (Aldrich 28,125-5, 27,529-8, 27,527-1); (7) dihydroxy phenylacetic acid (HO)<sub>2</sub>C<sub>6</sub>H<sub>3</sub>CH<sub>2</sub>COOH (Aldrich 16,868-8, 85,021-7); (8) bicine (HOCH<sub>2</sub>CH<sub>2</sub>)<sub>2</sub>NCH<sub>2</sub>COOH (Aldrich 16,379-1); (9) 2,2-bis(hydroxymethyl)propionic acid CH<sub>3</sub>C(CH<sub>2</sub>OH)<sub>2</sub>COOH (Aldrich 10,661-5); (10) 4,4-bis(4-hydroxyphenyl) valeric acid CH<sub>3</sub>C(C<sub>6</sub>H<sub>4</sub>OH)<sub>2</sub>CH<sub>2</sub>CH<sub>2</sub>COOH (Aldrich B4,770-7); (11) tris (hydroxymethyl) amino methane succinate [(HOCH<sub>2</sub>)<sub>3</sub>CNH<sub>2</sub>]<sub>2</sub>HOOCH<sub>2</sub>CH<sub>2</sub>COOH (Aldrich 34,068-5); and the like.

Polycarboxyl compounds generally are those compounds having at least two carboxyl functional groups. Examples of suitable polycarboxyl compounds include (I) aliphatic dicarboxy-functional compounds, including (a) compounds of the general formula HOOC(CH<sub>2</sub>)<sub>n</sub>COOH and their derivatives, wherein n represents the number of repeating units, including (1) [n=0], such as oxalic acid HOOCOOH, such as oxalic acid dihydrate HOOCOOH.2H<sub>2</sub>O (Aldrich 0-875-5); (2) [n=1], such as malonic acid HOOCC<sub>2</sub>COOH (Aldrich M129-6); (3) [n=2], such as succinic acid HOOC(CH<sub>2</sub>)<sub>2</sub>COOH (Aldrich 13,438-4); (4) [n=3], such as glutaric acid HOOC(CH<sub>2</sub>)<sub>3</sub>COOH (Aldrich G340-7); (5) [n=4], such as adipic acid HOOC(CH<sub>2</sub>)<sub>4</sub>COOH (Aldrich 24,052-4); (6) [n=5], such as pimelic acid HOOC(CH<sub>2</sub>)<sub>5</sub>COOH (Aldrich P4,500-1); (7) [n=6], such as suberic acid HOOC(CH<sub>2</sub>)<sub>6</sub>COOH (Aldrich S520-0); (8) [n=7], such as azelaic acid HOOC(CH<sub>2</sub>)<sub>7</sub>COOH (Aldrich A9,615-0); (9) [n=8], such as sebamic acid HOOC(CH<sub>2</sub>)<sub>8</sub>COOH (Aldrich S175-2); (10) [n=9], such as undecanedioic acid HOOC(CH<sub>2</sub>)<sub>9</sub>COOH (Aldrich 17,796-2); (11) [n=10], such as 1,10-decane dicarboxylic acid HOOC(CH<sub>2</sub>)<sub>10</sub>COOH (Aldrich D100-9); (12) [n=11], such as 1,11-undecane dicarboxylic acid HOOC(CH<sub>2</sub>)<sub>11</sub>COOH (Aldrich U60-1); (13) [n=12], such as 1,12,dodecane dicarboxylic acid HOOC(CH<sub>2</sub>)<sub>12</sub>COOH (Aldrich D22,120-1); (14) [n=14], such as hexadecanedioic acid HOOC(CH<sub>2</sub>)<sub>14</sub>COOH (Aldrich 17,750-4); (15) [n=22], such as tetracosane dioic acid HOOC(CH<sub>2</sub>)<sub>22</sub>COOH (Aldrich 30,670-3); derivatives of malonic acid, such as (16) methyl malonic acid HOOCC(CH<sub>3</sub>)COOH (Aldrich M5,405-8); (17) ketomalonic acid monohydrate HOOCC(OH)<sub>2</sub>COOH (Aldrich 16,343-0); (18) ethyl malonic acid HOOC(C<sub>2</sub>H<sub>5</sub>)COOH (Aldrich 10,268-7); (19) diethyl malonic acid HOOC(C<sub>2</sub>H<sub>5</sub>)<sub>2</sub>COOH (Aldrich 24,654-9); derivatives of succinic acid, such as (20) mercapto succinic acid HOOCCH<sub>2</sub>CH(SH)COOH (Aldrich M618-2); (21) methyl succinic acid HOOCCH<sub>2</sub>CH(CH<sub>3</sub>)COOH (Aldrich M8,120-9); (22) malic acid HOOCCH<sub>2</sub>CH(OH)COOH (Aldrich M121-0); (23) 2,3-dimethyl succinic acid HOOCCH(CH<sub>3</sub>)CH(CH<sub>3</sub>)COOH (Aldrich D18,620-1); (24) citramalic acid HOOCCH<sub>2</sub>C(CH<sub>3</sub>)(OH)COOH (Aldrich 32,914-2); (25) ( $\pm$ )-cyclohexyl succinic acid HOOCCH<sub>2</sub>C(C<sub>6</sub>H<sub>11</sub>)COOH (Aldrich 33,219-4); (26) ( $\pm$ )-2-(carboxymethyl thio) succinic acid HOOCCH<sub>2</sub>CH(SCH<sub>2</sub>COOH)COOH (Aldrich 28,238-3); (27) tartaric acid HOOCCH(OH)CH(OH)COOH (Aldrich T20-6, T40-0, T-10-9, 25,138-0); derivatives of glutaric acid, such as (28) 2,2-dimethyl glutaric acid HOOCCH<sub>2</sub>CH<sub>2</sub>C(CH<sub>3</sub>)<sub>2</sub>COOH (Aldrich 20,526-5); (29) 2,4-dimethyl glutaric acid HOOCCH(CH<sub>3</sub>)CH<sub>2</sub>CH(CH<sub>3</sub>)COOH (Aldrich 23,941-0); (30) 3,3-dimethyl glutaric acid

HOOCCH<sub>2</sub>C(CH<sub>3</sub>)<sub>2</sub>CH<sub>2</sub>COOH (Aldrich D15,940-9); (31) 2-methyl glutaric acid HOOCCH<sub>2</sub>CH<sub>2</sub>CH(CH<sub>3</sub>)COOH (Aldrich 12,986-0); (32) 3-methyl glutaric acid HOOCCH<sub>2</sub>CH(CH<sub>3</sub>)CH<sub>2</sub>COOH (Aldrich M4,760-4); (33) 3,3-tetramethylene glutaric acid HOOCCH<sub>2</sub>C<sub>5</sub>H<sub>8</sub>CH<sub>2</sub>COOH (Aldrich T2,190-3); (34) 3-phenyl glutaric acid HOOC<sub>2</sub>CCGH<sub>5</sub>CHCH<sub>2</sub>COOH (Aldrich P2,520-5); (35) 2-ketoglutamic acid HOOCCH<sub>2</sub>CH<sub>2</sub>COCOOH (Aldrich K160-0); (36) 3-keto-glutamic acid HOOCCH<sub>2</sub>COCH<sub>2</sub>COOH (Aldrich 16,511-5); derivatives of adipic acid, such as (37) 3-methyl adipic acid HOOC(CH<sub>2</sub>)<sub>2</sub>CH(CH<sub>3</sub>)CH<sub>2</sub>COOH (Aldrich M2,740-9); derivatives of pimelic acid, such as (38) ( $\pm$ )-2,6-diamino pimelic acid HOOCCH(NH<sub>2</sub>)(CH<sub>2</sub>)<sub>3</sub>CH(NH<sub>2</sub>)COOH (Aldrich 27,147-0); (39) 4-ketopimelic acid HOOCCH<sub>2</sub>CH<sub>2</sub>COCH<sub>2</sub>CH<sub>2</sub>COOH (Aldrich K350-6); other derivatives, such as (40) mucic acid (galactaric acid) HOOC(CHOH)<sub>4</sub>COOH (Aldrich M8,961-7); (41) 3-methylene cyclopropane-trans-1,2-dicarboxylic acid H<sub>2</sub>C=C(CHCOOH)<sub>2</sub> (Aldrich 22,053-1); (42) 1,1-cyclobutane dicarboxylic acid C<sub>4</sub>H<sub>6</sub>(COOH)<sub>2</sub> (Aldrich C9,580-3); (43) cyclohexane dicarboxylic acid C<sub>6</sub>H<sub>10</sub>(COOH)<sub>2</sub> (Aldrich 30,703-3, C10,075-7, 33,123-6); (b) compounds of the general formula R(CH<sub>2</sub>COOH)<sub>2</sub> and their derivatives, wherein R is selected from the group consisting of imine, acetamido imine, alkylimine, oxo, and cycloalkane, including (1) when R=NH, such as imino diacetic acid NH(CH<sub>2</sub>COOH)<sub>2</sub> (Aldrich 22,000-0); (2) when R=H<sub>2</sub>NCOCH<sub>2</sub>N, such as [N-(2-acetamido) imino diacetic acid] H<sub>2</sub>NCOCH<sub>2</sub>N(CH<sub>2</sub>COOH)<sub>2</sub> (Aldrich 85,760-2); (3) when R=CH<sub>3</sub>N, such as methyl iminodiacetic acid CH<sub>3</sub>N(CH<sub>2</sub>COOH)<sub>2</sub> (Aldrich M5,100-8); (4) when R=O, such as diglycolic acid O(CH<sub>2</sub>COOH)<sub>2</sub> (Aldrich 14,307-3); (5) when R=CGH<sub>10</sub>, such as 1,1-cyclohexane diacetic acid C<sub>6</sub>H<sub>10</sub>(CH<sub>2</sub>COOH)<sub>2</sub> (Aldrich 17,134-4); (c) compounds of the general formula HOOC(CH<sub>2</sub>)<sub>n</sub>CH=CHCOOH and their derivatives, wherein n represents the number of repeating units, including (1) [n=0], such as fumaric acid HOOCCH=CHCOOH (Aldrich 24,074-5, F1 935-3) and (2) maleic acid HOOC—CH=CH—COOH (Aldrich M15-3); (3) [n=1], such as glutamic acid HOOCCH<sub>2</sub>CH=CHCOOH (Aldrich G260-5); (4) [n=8], such as 2-dodecenedioic acid HOOC(CH<sub>2</sub>)<sub>8</sub>CH=CHCOOH (Aldrich 17,724-5); derivatives of fumaric or maleic acid, such as (5) mesaconic acid HOOCCH=C(CH<sub>3</sub>)COOH (Aldrich 13,104-6); (6) citraconic acid HOOC(CH<sub>3</sub>)C=CHCOOH (Aldrich C<sub>8</sub>,260-4); (7) dihydroxy fumaric acid hydrate HOOC(OH)=C(OH)COOH.xH<sub>2</sub>O (Aldrich D11,320-4); and other derivatives, such as (8) trans, trans-1,3-butadiene-1,4-dicarboxylic acid HOOCCH=CHCH=CHCOOH (Aldrich M9,000-3); and the like.

Also suitable are (II) aromatic dicarboxy-functional compounds, such as (1) homophthalic acid HOOCCH<sub>2</sub>C<sub>6</sub>H<sub>4</sub>COOH (Aldrich H<sub>1</sub>,620-5); (2) terephthalic acid C<sub>6</sub>H<sub>4</sub>-1,4-(COOH)<sub>2</sub> (Aldrich 18,536-1); (3) phthalic acid C<sub>6</sub>H<sub>4</sub>-1,2-(COOH)<sub>2</sub> (Aldrich P3,930-3); (4) 4-methyl phthalic acid CH<sub>3</sub>C<sub>6</sub>H<sub>3</sub>-1,2-(COOH)<sub>2</sub> (Aldrich 34,830-9); (5) chelidonic acid monohydrate (Aldrich 12,495-8), of the formula:



(6) chelidamic acid monohydrate (Aldrich C<sub>1,820-5</sub>), of the formula:



(7) cis-5-norbornene-endo-2,3-dicarboxylic acid (Aldrich 21,670-4), of the formula:



(8) 1,4-naphthalene dicarboxylic acid C<sub>10</sub>H<sub>6</sub>(COOH)<sub>2</sub> (Aldrich 33,358-1); (9) 2,3-naphthalene dicarboxylic acid C<sub>10</sub>H<sub>6</sub>(COOH)<sub>2</sub> (Aldrich N40-0); (10) 2,6-naphthalene dicarboxylic acid C<sub>10</sub>H<sub>6</sub>(COOH)<sub>2</sub> (Aldrich 30,153-3); (11) 4-carboxy phenoxy acetic acid HOOC<sub>6</sub>H<sub>4</sub>OCH<sub>2</sub>COOH (Aldrich 18,662-7); (12) 2,5-dihydroxy-1,4-benzene diacetic acid (HO)<sub>2</sub>C<sub>6</sub>H<sub>2</sub>(CH<sub>2</sub>COOH)<sub>2</sub> (Aldrich D10,920-7); (13) pamoic acid [4,4'-methylene bis (3-hydroxy-2-naphthoic acid)] (Aldrich P9-4), of the formula:



(14) 4-[4-(2-carboxybenzoyl) phenyl] butyric acid HOOCC<sub>6</sub>H<sub>4</sub>COC<sub>6</sub>H<sub>4</sub> (CH<sub>2</sub>)<sub>3</sub>COOH (Aldrich 19,281-3); (15) 1,4-phenylene diacrylic acid HOOCH=CHC<sub>6</sub>H<sub>4</sub>CH=CHCOOH (Aldrich P2,390-3); (16) 2-carboxy cinnamic acid HOOCC<sub>6</sub>H<sub>4</sub>CH=CHCOOH (Aldrich 18,603-1); (17)  $\gamma$ -L-glutamyl-L-cysteinyl glycine HOOCCH(NH<sub>2</sub>)CH<sub>2</sub>CH<sub>2</sub>CONHCH(CH<sub>2</sub>SH)CONHCH<sub>2</sub>COOH (Aldrich G470-5); (18) D,L-isocitriclactone [DL-2-oxotetrahydrofuran-2,3,4,5-tetracarboxylic acid (Aldrich I-1,600-5), of the formula:



(19) N-(2-hydroxyethyl) iminodiacetic acid HOCH<sub>2</sub>CH<sub>2</sub>N(CH<sub>2</sub>COOH)<sub>2</sub> (Aldrich 15,814-3); (20) dipivaloyl-L-tartaric acid (Aldrich 33,788-9); (21) ( $\pm$ )-cyclohexyl succinic acid HOOCH<sub>2</sub>CH(C<sub>6</sub>H<sub>11</sub>)COOH (Aldrich 33,219-4); (22) phenyl diacetic acid C<sub>6</sub>H<sub>4</sub>(CH<sub>2</sub>COOH)<sub>2</sub> (Aldrich 13,140-7, P2,335-0, P2,340-7); and the like.

Also suitable are (III) aliphatic and aromatic compounds with more than two —COOH functional groups, including (1) 1,3,5-cyclohexane tricarboxylic acid C<sub>6</sub>H<sub>9</sub>(COOH)<sub>3</sub> (Aldrich 34,434-6); (2) citric acid monohydrate HOOCH<sub>2</sub>C(OH)(COOH)CH<sub>2</sub>COOH.H<sub>2</sub>O (Aldrich 24,752-9); (3) 1,2,3-propene tricarboxylic acid HOOCH=CH(COOH)CH<sub>2</sub>COOH (Aldrich 27,194-2); (4) 1,2,3-propane tricarboxylic acid HOOCH<sub>2</sub>CH(COOH)CH<sub>2</sub>COOH (Aldrich T-5,350-3); (5)  $\beta$ -methyl tricarballycic acid HOOCH<sub>2</sub>C(CH<sub>3</sub>)<sub>2</sub>COOHCH<sub>2</sub>COOH (Aldrich M8,520-4); (6) 1,2,3,4-cyclobutane tetracarboxylic acid C<sub>4</sub>H<sub>4</sub>(COOH)<sub>4</sub> (Aldrich 32,494-9); (7) 1,2-diaminocyclohexane-N,N,N',N'-tetraacetic acid hydrate C<sub>6</sub>H<sub>10</sub>[N(CH<sub>2</sub>COOH)<sub>2</sub>]<sub>2</sub>.xH<sub>2</sub>O (Aldrich 12581-4); (8) 1,6-diaminohexane-N,N,N',N'-tetraacetic acid hydrate (HOOCH<sub>2</sub>)<sub>2</sub>N(CH<sub>2</sub>)<sub>6</sub>N(CH<sub>2</sub>COOH)<sub>2</sub>.xH<sub>2</sub>O (Aldrich 23,245-9); (9) 1,2,4,5-benzene tetracarboxylic acid C<sub>6</sub>H<sub>2</sub>(COOH)<sub>4</sub> (Aldrich B,400-7); (10) 1,4,5,8-naphthalene tetracarboxylic acid hydrate C<sub>10</sub>H<sub>4</sub>(COOH)<sub>4</sub>.xH<sub>2</sub>O (Aldrich 13009-5); (11) penta diethylene triamine penta acetic acid (HOOCH<sub>2</sub>)<sub>2</sub>NCH<sub>2</sub>CH<sub>2</sub>(CH<sub>2</sub>COOH)CH<sub>2</sub>CH<sub>2</sub>N(CH<sub>2</sub>COOH)<sub>2</sub> (Aldrich 28,556-0, D9,390-2); (12) mellitic acid C<sub>6</sub>(COOH)<sub>6</sub> (Aldrich M270-5); (13) agaricic acid (2-hydroxy-1,2,3-nonadecane tricarboxylic acid) CH<sub>3</sub>(CH<sub>2</sub>)<sub>15</sub>CH(COOH)C(OH)(COOH)CH<sub>2</sub>COOH (Aldrich 21,783-2); (14) 1,2-diamino propane-N,N,N',N'-tetraacetic acid (HOOCH<sub>2</sub>)NCH(CH<sub>3</sub>)CH<sub>2</sub>N(CH<sub>2</sub>COOH)<sub>2</sub> (Aldrich 15,813-5); (15) ethylene diamine tetraacetic acid (HOOCH<sub>2</sub>)<sub>2</sub>NCH<sub>2</sub>CH<sub>2</sub>N(CH<sub>2</sub>COOH)<sub>2</sub> (Aldrich 25,404-5); (16) ( $\pm$ )-2-(carboxymethylthio) succinic acid HOOCH<sub>2</sub>CH(SCH<sub>2</sub>COOH)COOH (Aldrich 28,238-3); (17) N-(2-hydroxyethyl) ethylene diamine triacetic acid HOCH<sub>2</sub>CH<sub>2</sub>N(CH<sub>2</sub>COOH)CH<sub>2</sub>CH<sub>2</sub>N(CH<sub>2</sub>COOH)<sub>2</sub> (Aldrich H<sub>2</sub>,650-1); (18) N,N'-bis(2-carboxyethyl)-N,N'-ethylene di glycine trihydrate [—CH<sub>2</sub>N(CH<sub>2</sub>COOH)CH<sub>2</sub>CH<sub>2</sub>COOH]<sub>2</sub>.3H<sub>2</sub>O; (19) tetrahydrofuran-2,3,4,5-tetracarboxylic acid (Aldrich 14,483-5), of the formula:



and the like.

Mixtures of two or more of any of the above compounds can also be employed.

The amino acid, hydroxy acid, polycarboxyl compound, or mixture thereof is present in any effective amount relative to the substrate. Typically, the amino acid, hydroxy acid, polycarboxyl compound, or mixture thereof is present in an

amount of from about 1 to about 50 percent by weight of the substrate, preferably from about 5 to about 30 percent by weight of the substrate, although the amount can be outside this range. The amount can also be expressed in terms of the weight of amino acid, hydroxy acid, polycarboxyl compound, or mixture thereof per unit area of substrate. Typically, the amino acid, hydroxy acid, polycarboxyl compound, or mixture thereof is present in an amount of from about 0.8 to about 40 grams per square meter of the substrate surface to which it is applied, and preferably from about 4 to about 24 grams per square meter of the substrate surface to which it is applied, although the amount can be outside these ranges.

When the amino acid, hydroxy acid, polycarboxyl compound, or mixture thereof is applied to the substrate as a coating, the coatings employed for the recording sheets of the present invention can include an optional binder in addition to the amino acid, hydroxy acid, polycarboxyl compound, or mixture thereof. Examples of suitable binder polymers include (a) hydrophilic polysaccharides and their modifications, such as (1) starch (such as starch SLS-280, available from St. Lawrence starch), (2) cationic starch (such as Cato-72, available from National Starch), (3) hydroxyalkylstarch, wherein alkyl has at least one carbon atom and wherein the number of carbon atoms is such that the material is water soluble, preferably from about 1 to about 20 carbon atoms, and more preferably from about 1 to about 10 carbon atoms, such as methyl, ethyl, propyl, butyl, or the like (such as hydroxypropyl starch (#02382, available from Poly Sciences Inc.) and hydroxyethyl starch (#06733, available from Poly Sciences Inc.)), (4) gelatin (such as Calfskin gelatin #00639, available from Poly Sciences Inc.), (5) alkyl celluloses and aryl celluloses, wherein alkyl has at least one carbon atom and wherein the number of carbon atoms is such that the material is water soluble, preferably from 1 to about 20 carbon atoms, more preferably from 1 to about 10 carbon atoms, and even more preferably from 1 to about 7 carbon atoms, such as methyl, ethyl, propyl, butyl, pentyl, hexyl, benzyl, and the like (such as methyl cellulose (Methocel AM 4, available from Dow Chemical Company)), and wherein aryl has at least 6 carbon atoms and wherein the number of carbon atoms is such that the material is water soluble, preferably from 6 to about 20 carbon atoms, more preferably from 6 to about 10 carbon atoms, and even more preferably about 6 carbon atoms, such as phenyl, (6) hydroxy alkyl celluloses, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as hydroxyethyl cellulose (Natrosol 250 LR, available from Hercules Chemical Company), and hydroxypropyl cellulose (Klucel Type E, available from Hercules Chemical Company)), (7) alkyl hydroxy alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as ethyl hydroxyethyl cellulose (Bermocoll, available from Berol Kem. A. B. Sweden)), (8) hydroxy alkyl alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as hydroxyethyl methyl cellulose (HEM,

available from British Celanese Ltd., also available as Tylose MH, MHK from Kalle A. G.), hydroxypropyl methyl cellulose (Methocel K35LV, available from Dow Chemical Company), and hydroxy butylmethyl cellulose (such as HBMC, available from Dow Chemical Company)), (9) dihydroxyalkyl cellulose, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dihydroxypropyl cellulose, which can be prepared by the reaction of 3-chloro-1,2-propane with alkali cellulose), (10) hydroxy alkyl hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxypropyl hydroxyethyl cellulose, available from Aqualon Company), (11) halodeoxycellulose, wherein halo represents a halogen atom (such as chlorodeoxycellulose, which can be prepared by the reaction of cellulose with sulfonyl chloride in pyridine at 25° C.), (12) amino deoxycellulose (which can be prepared by the reaction of chlorodeoxy cellulose with 19 percent alcoholic solution of ammonia for 6 hours at 160° C.), (13) dialkylammonium halide hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as diethylammonium chloride hydroxy ethyl cellulose, available as Celquat H-100, L-200, National Starch and Chemical Company), (14) hydroxyalkyl trialkyl ammonium halide hydroxyalkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as hydroxypropyl trimethyl ammonium chloride hydroxyethyl cellulose, available from Union Carbide Company as Polymer JR), (15) dialkyl amino alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, (such as diethyl amino ethyl cellulose, available from Poly Sciences Inc. as DEAE cellulose #05178), (16) carboxyalkyl dextrans, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, and the like, (such as carboxymethyl alextrans, available from Poly Sciences Inc. as #16058), (17) dialkyl aminoalkyl dextran, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as diethyl aminoethyl dextran, available from Poly Sciences Inc. as #5178), (18) amino dextran (available from Molecular Probes Inc), (19) carboxy alkyl cellulose salts, wherein alkyl has at least one carbon atom and wherein the number of carbon atoms is such that the material is water soluble, preferably from 1 to

about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethyl cellulose CMC 7HOF, available from Hercules Chemical Company), (20) gum arabic (such as #69752, available from Sigma Chemical Company), (21) carrageenan (such as #C<sub>1013</sub> available from Sigma Chemical Company), (22) Karaya gum (such as #(30503, available from Sigma Chemical Company), (23) xanthan (such as Keltrol-T, available from Kelco division of Merck and Company), chitosan (such as #C3646, available from Sigma Chemical Company), (25) carboxyalkyl hydroxyalkyl guar, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as carboxymethyl hydroxypropyl guar, available from Aqualon Company), (26) cationic guar (such as Celanese Jaguars C-14-S, C-15, C-17, available from Celanese Chemical Company), (27) n-carboxyalkyl chitin, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, such as n-carboxymethyl chitin, (28) dialkyl ammonium hydrolyzed collagen protein, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dimethyl ammonium hydrolyzed collagen protein, available from Croda as Croquats), (29) agar-agar (such as that available from Pfaltz and Bauer Inc), (30) cellulose sulfate salts, wherein the cation is any conventional cation, such as sodium, lithium, potassium, calcium, magnesium, or the like (such as sodium cellulose sulfate #023 available from Scientific Polymer Products), and (31) carboxyalkylhydroxyalkyl cellulose salts, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethylhydroxyethyl cellulose CMHEC 43H and 37L available from Hercules Chemical Company); (b) vinyl polymers, such as (1) poly(vinyl alcohol) (such as Elvanol available from Dupont Chemical Company), (2) poly (vinyl phosphate) (such as #4391 available from Poly Sciences Inc.), (3) poly (vinyl pyrrolidone) (such as that available from GAF Corporation), (4) vinyl pyrrolidone-vinyl acetate copolymers (such as #02587, available from Poly Sciences Inc.), (5) vinyl pyrrolidone-styrene copolymers (such as #371, available from Scientific Polymer Products), (6) poly (vinylamine) (such as #1562, available from Poly Sciences Inc.), (7) poly (vinyl alcohol) alkoxylated, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl alcohol) ethoxylated #6573, available from Poly Sciences Inc.), and (8) poly (vinyl pyrrolidone-dialkylaminoalkyl alkylacrylate), wherein each alkyl has at least one carbon atom and wherein the number

of carbon atoms is such that the material is water soluble, preferably from 1 to about 20 carbon atoms, more preferably from 1 to about 10 carbon atoms, such as methyl, ethyl, propyl, butyl, and the like (such as poly (vinyl pyrrolidone-diethylaminomethylmethacrylate) #16294 and #16295, available from Poly Sciences Inc.); (c) formaldehyde resins, such as (1) melamine-formaldehyde resin (such as BC 309, available from British Industrial Plastics Limited), (2) urea-formaldehyde resin (such as BC<sub>777</sub>, available from British Industrial Plastics Limited), and (3) alkylated urea-formaldehyde resins, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methylated urea-formaldehyde resins, available from American Cyanamid Company as Beetle 65); (d) ionic polymers, such as (1) poly (2-acrylamide-2-methyl propane sulfonic acid) (such as #175 available from Scientific Polymer Products), (2) poly (N,N-dimethyl-3,5-dimethylene piperidinium chloride) (such as #401, available from Scientific Polymer Products), and (3) poly (methylene-guanidine) hydrochloride (such as #654, available from Scientific Polymer Products); (e) latex polymers, such as (1) cationic, anionic, and nonionic styrene-butadiene latexes (such as that available from Gen Corp Polymer Products, such as RES 4040 and RES 4100, available from Unocal Chemicals, and such as DL 6672A, DL6638A, and DL6663A, available from Dow Chemical Company), (2) ethylenevinylacetate latex (such as Airflex 400, available from Air Products and Chemicals Inc.), (3) vinyl acetate-acrylic copolymer latexes (such as synthemul 97-726, available from Reichhold Chemical Inc, Resyn 25-1110 and Resyn 25-1140, available from National Starch Company, and RES 3103 available from Unocal Chemicals, (4) quaternary acrylic copolymer latexes, particularly those of the formula



wherein n is a number from about 10 to about 100, and preferably about 50, R is hydrogen or methyl, R<sub>1</sub> is hydrogen, an alkyl group, or an aryl group, and R<sub>2</sub> is N<sup>+</sup>(CH<sub>3</sub>)<sub>3</sub>X<sup>-</sup>, wherein X is an anion, such as Cl, Br, I, HSO<sub>3</sub>, SO<sub>3</sub>, CH<sub>2</sub>SO<sub>3</sub>, H<sub>2</sub>PO<sub>4</sub>, HPO<sub>4</sub>, PO<sub>4</sub>, or the like, and the degree of quaternization is from about 1 to about 100 percent, including polymers such as polymethyl acrylate trimethyl ammonium chloride latex, such as HX42-1, available from Interpolymer Corp., or the like; (f) maleic anhydride and maleic acid containing polymers, such as (1) styrene-maleic anhydride copolymers (such as that available as Scriptet from Monsanto, and the SMA series available from Arco), (2) vinyl alkyl ether-maleic anhydride copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinyl methyl ether-maleic anhydride copolymer #173, available from Scientific Polymer Products), (3) alkylene-maleic anhydride copolymers, wherein alkylene has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as ethylene-maleic anhydride copolymer #2308, available from Poly Sciences Inc., also available as EMA from Monsanto Chemical Com-

pany), (4) butadiene-maleic acid copolymers (such as #07787, available from Poly Sciences Inc.), (5) vinylalkyl-ether-maleic acid copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinylmethylether-maleic acid copolymer, available from GAF Corporation as Gantrez S-95), and (6) alkyl vinyl ether-maleic acid esters, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methyl vinyl ether-maleic acid ester #773, available from Scientific Polymer Products); (g) acrylamide containing polymers, such as (1) poly (acrylamide) (such as #02806, available from Poly Sciences Inc.), (2) acrylamide-acrylic acid copolymers (such as #04652, #02220, and #18545, available from Poly Sciences Inc.), and (3) poly (N,N-dimethyl acrylamide) (such as #004590, available from Poly Sciences Inc.); and (h) poly (alkylene imine) containing polymers, wherein alkylene has two (ethylene), three (propylene), or four (butylene) carbon atoms, such as (1) poly(ethylene imine) (such as #135, available from Scientific Polymer Products), (2) poly(ethylene imine) epichlorohydrin (such as #634, available from Scientific Polymer Products), and (3) alkoxylated poly (ethylene imine), wherein alkyl has one (methoxylated), two (ethoxylated), three (propoxylated), or four (butoxylated) carbon atoms (such as ethoxylated poly (ethylene imine) #636, available from Scientific Polymer Products); and the like, as well as blends or mixtures of any of the above, with starches and latexes being particularly preferred because of their availability and applicability to paper. Any mixtures of the above ingredients in any relative amounts can be employed.

If present, the binder can be present within the coating in any effective amount; typically the binder and the amino acid, hydroxy acid, polycarboxyl compound, or mixture thereof are present in relative amounts of from about 10 percent by weight binder and about 90 percent by weight amino acid, hydroxy acid, polycarboxyl compound, or mixture thereof to about 99 percent by weight binder and about 1 percent by weight amino acid, hydroxy acid, polycarboxyl compound, or mixture thereof, although the relative amounts can be outside of this range.

In addition, the coating of the recording sheets of the present invention can contain optional antistatic agents. Any suitable or desired antistatic agent or agents can be employed, such as quaternary salts and other materials as disclosed in, for example, copending applications 08/034, 917, and U.S. Pat. Nos. 5,314,747, 5,441,795, 5,320,902 and 5,457,486, disclosures of each of which are totally incorporated herein by reference. The antistatic agent can be present in any effective amount; typically, the antistatic agent is present in an amount of from about 1 to about 5 percent by weight of the coating, and preferably in an amount of from about 1 to about 2 percent by weight of the coating, although the amount can be outside these ranges.

Further, the coating of the recording sheets of the present invention can contain one or more optional biocides. Examples of suitable biocides include (A) non-ionic biocides, such as (1) 2-hydroxypropylmethane thiosulfonate (Busan 1005, available from Buckman Laboratories Inc.); (2) 2-(thio cyanomethyl thio) benzothiazole (Busan 30WB, 72WB, available from Buckman Laboratories Inc.); (3) methylene bis (thiocyanate) (Metasol T-10, available from

Calgon Corporation; AMA-110, available from Vinings Chemical Company; Viehem MBT, available from Vineland Chemical Company; Aldrich 10,509-0); (4) 2-bromo-4'-hydroxyacetophenone (Busan 90, available from Buckman Laboratories); (5) 1,2-dibromo-2,4-dicyano-butane (Metasol CB-210, CB-235, available from Calgon Corporation); (6) 2,2-dibromo-3-nitropropionamide (Metasol RB-20, available from Calgon Corporation; Amerstat 300, available from Drew Industrial Div.); (7) N- $\alpha$ -(1-nitroethyl benzyl-ethylene diamine) (Metasol J-26, available from Calgon Corporation); (8) dichlorophene (G-4, available from Givaudan Corporation); (9) 3,5-dimethyl tetrahydro-2H-1, 3,5-thiadiazine-2-thione (SLIME-TROL RX-28, available from Betz Paper Chem Inc.); Metasol D3T-A, available from Calgon Corporation; SLIME ARREST, available from Western Chemical Company); (10) a non-ionic blend of a sulfone, such as bis (trichloromethyl) sulfone and methylene bisthiocyanate (available as SLIME-TROL RX-38A from Betz Paper Chem Inc.); (11) a non-ionic blend of methylene bisthiocyanate and bromonitrostyrene (available as SLIME-TROL RX-41 from Betz Paper Chem Inc.); (12) a non-ionic blend of 2-(thiocyanomethylthio) benzothiazole (53.2% by weight) and 2-hydroxypropyl methanethiosulfonate (46.8% by weight) (available as BUSAN 25 from Buckman Laboratories Inc.); (13) a non-ionic blend of methylene bis(thiocyanate) 50 percent by weight and 2-(thiocyanomethylthio) benzothiazole 50 percent by weight (available as BUSAN 1009, 1009WB from Buckman Laboratories Inc.); (14) a non-ionic blend of 2-bromo-4'-hydroxyacetophenone (70 percent by weight) and 2-(thiocyanomethylthio) benzothiazole (30 percent by weight) (BUSAN 93, available from Buckman Laboratories Inc.); (15) a non-ionic blend of 5-chloro-2-methyl-4-isothiazoline-3-one (75 percent by weight) and 2-methyl-4-isothiazolin-3-one (25 percent by weight), (available as AMERSTAT 250 from Drew Industrial Division; NALCON 7647, from NALCO Chemical Company; Kathon LY, from Rohm and Haas Co.); and the like, as well as mixtures thereof; (B) anionic biocides, such as (1) anionic potassium N-hydroxymethyl-N-methyl-dithiocarbamate (available as BUSAN 40 from Buckman Laboratories Inc.); (2) an anionic blend of N-hydroxymethyl-N-methyl dithiocarbamate (80% by weight) and sodium 2-mercapto benzothiazole (20% by weight) (available as BUSAN 52 from Buckman Laboratories Inc.); (3) an anionic blend of sodium dimethyl dithiocarbamate 50 percent by weight and (disodium ethylenebis-dithiocarbamate) 50% by weight (available as METASOL 300 from Calgon Corporation; AMERSTAT 272 from Drew Industrial Division; SLIME CONTROL F from Western Chemical Company); (4) an anionic blend of N-methyl dithiocarbamate 60 percent by weight and disodium cyanodithioimidocarbonate 40 percent by weight (available as BUSAN 881 from Buckman Laboratories Inc.); (5) An anionic blend of methylene bis-thiocyanate (33% by weight), sodium dimethyl-dithiocarbamate (33% by weight), and sodium ethylene bisdithiocarbamate (33% by weight) (available as AMERSTAT 282 from Drew Industrial Division; AMA-131 from Vinings Chemical Company); (6) sodium dichlorophene (G-4-40, available from Givaudan Corp.); and the like, as well as mixtures thereof; (C) cationic biocides, such as (1) cationic poly (oxyethylene (dimethylamino)-ethylene (dimethylamino) ethylene dichloride) (Busan 77, available from Buckman Laboratories Inc.); (2) a cationic blend of methylene bisthiocyanate and dodecyl guanidine hydrochloride (available as SLIME TROL RX-31, RX-32, RX-32P, RX-33, from Betz Paper Chem Inc.); (3) a cationic blend of a sulfone, such as bis(trichloromethyl) sulfone and a qua-

ternary ammonium chloride (available as SLIME TROL RX-36 DPB-865 from Betz Paper Chem. Inc.); (4) a cationic blend of methylene bis thiocyanate and chlorinated phenols (available as SLIME-TROL RX-40 from Betz Paper Chem Inc.); and the like, as well as mixtures thereof. The biocide can be present in any effective amount; typically, the biocide is present in an amount of from about 10 parts per million to about 3 percent by weight of the coating, although the amount can be outside this range.

Additionally, the coating of the recording sheets of the present invention can contain optional filler components. Fillers can be present in any effective amount, and if present, typically are present in amounts of from about 1 to about 60 percent by weight of the coating composition. Examples of 10 filler components include colloidal silicas, such as Syloid 74, available from Grace Company (preferably present, in one embodiment, in an amount of about 20 weight percent), titanium dioxide (available as Rutile or Anatase from NL Chem Canada, Inc.), hydrated alumina (Hydrad TMC-HBF, 15 Hydrad TM-HBC, available from J.M. Huber Corporation), barium sulfate (K.C. Blanc Fix HD80, available from Kali Chemie Corporation), calcium carbonate (Microwhite Sylacauga Calcium Products), high brightness clays (such as Engelhard Paper Clays), calcium silicate (available from J.M. Huber Corporation), cellulosic materials insoluble in 20 water or any organic solvents (such as those available from Scientific Polymer Products), blend of calcium fluoride and silica, such as Opalex-C available from Kemira.O.Y, zinc oxide, such as Zoco Fax 183, available from Zo Chem, blends of zinc sulfide with barium sulfate, such as Lithopane, available from Schtебen Company, and the like, as 25 well as mixtures thereof. Brightener fillers can enhance color mixing and assist in improving print-through in recording sheets of the present invention.

The coating containing the amino acid, hydroxy acid, polycarboxyl compound, or mixture thereof is present on the substrate of the recording sheet of the present invention in any effective thickness. Typically, the total thickness of the 30 coating layer (on each surface, when both sides of the substrate are coated) is from about 1 to about 25 microns and preferably from about 5 to about 10 microns, although the thickness can be outside of these ranges.

The amino acid, hydroxy acid, polycarboxyl compound, or mixture thereof, or the mixture of amino acid, hydroxy acid, polycarboxyl compound, or mixture thereof with an optional binder, optional antistatic agent, optional biocide, and/or optional filler can be applied to the substrate by any suitable technique, such as size press treatment, dip coating, reverse roll coating, extrusion coating, or the like. For example, the coating can be applied with a KRK size press (Kumagai Riki Kogyo Co., Ltd., Nerima, Tokyo, Japan) by dip coating and can be applied by solvent extrusion on a Faustel Coater. The KRK size press is a lab size press that simulates a commercial size press. This size press is normally sheet fed, whereas a commercial size press typically employs a continuous web. On the KRK size press, the substrate sheet is taped by one end to the carrier mechanism plate. The speed of the test and the roll pressures are set, and the coating solution is poured into the solution tank. A 4 liter stainless steel beaker is situated underneath for retaining the solution overflow. The coating solution is cycled once through the system (without moving the substrate sheet) to wet the surface of the rolls and then returned to the feed tank, where it is cycled a second time. While the rolls are being "wetted", the sheet is fed through the sizing rolls by pressing the carrier mechanism start button. The coated sheet is then removed from the carrier mechanism plate and is placed on

a 12 inch by 40 inch sheet of 750 micron thick Teflon for support and is dried on the Dynamic Former drying drum and held under restraint to prevent shrinkage. The drying temperature is approximately 105° C. This method of coating treats both sides of the substrate simultaneously.

In dip coating, a web of the material to be coated is transported below the surface of the liquid coating composition by a single roll in such a manner that the exposed site is saturated, followed by removal of any excess coating by the squeeze rolls and drying at 100° C. in an air dryer. The liquid coating composition generally comprises the desired coating composition dissolved in a solvent such as water, methanol, or the like. The method of surface treating the substrate using a coater results in a continuous sheet of substrate with the coating material applied first to one side and then to the second side of this substrate. The substrate can also be coated by a slot extrusion process, wherein a flat die is situated with the die lips in close proximity to the web of substrate to be coated, resulting in a continuous film of the coating solution evenly distributed across one surface of the sheet, followed by drying in an air dryer at 100° C.

Recording sheets of the present invention can be employed in ink jet printing processes. One embodiment of the present invention is directed to a process which comprises applying an aqueous recording liquid to a recording sheet of the present invention in an imagewise pattern. Another embodiment of the present invention is directed to a printing process which comprises (1) incorporating into an ink jet printing apparatus containing an aqueous ink a recording sheet of the present invention, and (2) causing droplets of the ink to be ejected in an imagewise pattern onto the recording sheet, thereby generating images on the recording sheet. Ink jet printing processes are well known, and are described in, for example, U.S. Pat. No. 4,601,777, U.S. Pat. No. 4,251,824, U.S. Pat. No. 4,410,899, U.S. Pat. No. 4,412,224, and U.S. Pat. No. 4,532,530, the disclosures of each of which are totally incorporated herein by reference. In a particularly preferred embodiment, the printing apparatus employs a thermal ink jet process wherein the ink in the nozzles is selectively heated in an imagewise pattern, thereby causing droplets of the ink to be ejected in image-wise pattern. In another preferred embodiment, the substrate is printed with an aqueous ink and thereafter the printed substrate is exposed to microwave radiation, thereby drying the ink on the sheet. Printing processes of this nature are disclosed in, for example, U.S. Pat. No. 5,220,346, the disclosure of which is totally incorporated herein by reference.

The recording sheets of the present invention can also be used in any other printing or imaging process, such as printing with pen plotters, handwriting with ink pens, offset printing processes, or the like, provided that the ink employed to form the image is compatible with the ink receiving layer of the recording sheet.

Recording sheets of the present invention exhibit reduced curl upon being printed with aqueous inks, particularly in situations wherein the ink image is dried by exposure to microwave radiation. Generally, the term "curl" refers to the distance between the base line of the arc formed by recording sheet when viewed in cross-section across its width (or shorter dimension—for example, 8.5 inches in an 8.5×11 inch sheet, as opposed to length, or longer dimension—for example, 11 inches in an 8.5×11 inch sheet) and the midpoint of the arc. To measure curl, a sheet can be held with the thumb and forefinger in the middle of one of the long edges of the sheet (for example, in the middle of one of the 11 inch edges in an 8.5×11 inch sheet) and the arc formed by

the sheet can be matched against a pre-drawn standard template curve.

Specific embodiments of the invention will now be described in detail. These examples are intended to be illustrative, and the invention is not limited to the materials, conditions, or process parameters set forth in these embodiments. All parts and percentages are by weight unless otherwise indicated.

The optical density measurements recited herein were obtained on a Pacific Spectrograph Color System. The system consists of two major components, an optical sensor and a data terminal. The optical sensor employs a 6 inch integrating sphere to provide diffuse illumination and 8 degrees viewing. This sensor can be used to measure both transmission and reflectance samples. When reflectance samples are measured, a specular component may be included. A high resolution, full dispersion, grating monochromator was used to scan the spectrum from 380 to 720 nanometers. The data terminal features a 12 inch CRT display, numerical keyboard for selection of operating parameters and the entry of tristimulus values, and an alphanumeric keyboard for entry of product standard information.

#### EXAMPLE I

Transparency sheets were prepared as follows. Blends of 70 percent by weight hydroxypropyl methyl cellulose (K35LV, obtained from Dow Chemical Co.) and 30 percent by weight of various additive compositions, each obtained from Aldrich Chemical Co., were prepared by mixing 56

Cyan: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co., 30 percent by weight Projet Cyan 1 dye, obtained from ICI, 45.45 percent by weight water.

Magenta: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co., 2.5 percent by weight Triton Direct Red 227, obtained from Tricon, 72.95 percent by weight water.

Yellow: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co., 3 percent by weight Hoechst Duasyn Brilliant Yellow SF-GL VP220, obtained from Hoechst, 72.45 percent by weight water.

Images were generated by printing block patterns for magenta, cyan, yellow, and black. The images thus formed were dried by exposure to microwave radiation with a Citizen Model No. JM55581, obtained from Consumers, Mississauga, Ontario, Canada, set at 700 Watts output power at 2450 MHz frequency. The black images were "process black" (i.e., formed by superimposition of cyan, magenta, and yellow images). The drying times and optical densities for the resulting images were as follows:

| Additive                 | Drying Time (seconds) |      |         |        | Optical Density |      |         |        |
|--------------------------|-----------------------|------|---------|--------|-----------------|------|---------|--------|
|                          | black                 | cyan | magenta | yellow | black           | cyan | magenta | yellow |
| none                     | 30                    | 20   | 30      | 20     | 2.50            | 2.07 | 1.45    | 0.99   |
| D,L-2-amino butyric acid | 20                    | 30   | 30      | 20     | 1.70            | 1.70 | 1.50    | 0.98   |
| L-arginine hydrochloride | 10                    | 30   | 30      | 30     | 1.80            | 2.10 | 1.65    | 0.95   |
| N-acetyl-D,L-methionine  | 10                    | 40   | 10      | 20     | 1.88            | 1.70 | 1.49    | 0.94   |
| L-tartaric acid          | 20                    | 20   | 30      | 30     | 2.00            | 1.80 | 1.41    | 0.87   |
| 3-hydroxy benzoic acid   | 20                    | 20   | 25      | 20     | 1.95            | 1.80 | 1.45    | 0.92   |

grams of hydroxypropyl methyl cellulose and 24 grams of the additive composition in 1,000 milliliters of water in a 2 Liter jar and stirring the contents in an Omni homogenizer for 2 hours. Subsequently, the solution was left overnight for removal of air bubbles. The blends thus prepared were then coated by a dip coating process (both sides coated in one operation) by providing Mylar® base sheets in cut sheet form (8.5x11 inches) in a thickness of 100 microns. Subsequent to air drying at 25° C. for 3 hours followed by oven drying at 100° C. for 10 minutes and monitoring the difference in weight prior to and subsequent to coating, the dried coated sheets were each coated with 1 gram, 10 microns in thickness, on each surface (2 grams total coating weight for 2-sided transparency) of the substrate. For comparison purposes, a transparency sheet was also prepared in which the coating consisted of 100 percent by weight hydroxypropyl methyl cellulose and contained no additive composition.

The transparency sheets thus prepared were incorporated into a Hewlett-Packard 500-C color ink jet printer containing inks of the following compositions:

As the results indicate, the drying times for the process black images in all cases was faster in the presence of the additives than in their absence. In addition, all of the images exhibited acceptable optical densities.

#### EXAMPLE II

Transparency sheets were prepared as follows. Blends of 90 percent by weight hydroxypropyl methyl cellulose (K35LV, obtained from Dow Chemical Co.) and 10 percent by weight of various additive compositions, each obtained from Aldrich Chemical Co., were prepared by mixing 72 grams of hydroxypropyl methyl cellulose and 8 grams of the additive composition in 1,000 milliliters of water in a 2 Liter jar and stirring the contents in an Omni homogenizer for 2 hours. Subsequently, the solution was left overnight for removal of air bubbles. The blends thus prepared were then coated by a dip coating process (both sides coated in one operation) by providing Mylar® base sheets in cut sheet form (8.5x11 inches) in a thickness of 100 microns. Subsequent to air drying at 25° C. for 3 hours followed by oven drying at 100° C. for 10 minutes and monitoring the differ-

ence in weight prior to and subsequent to coating, the dried coated sheets were each coated with 1 gram, 10 microns in thickness, on each surface (2 grams total coating weight for 2-sided transparency) of the substrate. For comparison purposes, a transparency sheet was also prepared in which the coating consisted of 100 percent by weight hydroxypropyl methyl cellulose and contained no additive composition.

The transparency sheets thus prepared were incorporated into a Hewlett-Packard 500-C color ink jet printer containing inks of the following compositions:

Cyan: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 30 percent by weight Projet Cyan 1 dye, obtained from ICI, 45.45 percent by weight water.

Magenta: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 2.5 percent by weight Triton Direct Red 227, obtained from Tricon, 72.95 percent by weight water.

Yellow: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 3 percent by weight Hoechst Duasyn Brilliant Yellow SF-GL VP220, obtained from Hoechst, 72.45 percent by weight water.

Images were generated by printing block patterns for magenta, cyan, yellow, and black. The images thus formed were allowed to dry at 25° C. The black images were "process black" (i.e., formed by superimposition of cyan, magenta, and yellow images). The drying times and optical densities for the resulting images were as follows:

each obtained from Aldrich Chemical Co., were prepared by dissolving 50 grams of the additive in 500 milliliters of water in a beaker and stirring for 1 hour at 25° C. The additive solutions thus prepared were then coated onto paper by a dip coating process (both sides coated in one operation) by providing paper base sheets in cut sheet form (8.5×11 inches) in a thickness of 100 microns. Subsequent to air drying at 100° C. for 10 minutes and monitoring the difference in weight prior to and subsequent to coating, the sheets were each coated on each side with 500 milligrams, in a thickness of 5 microns (total coating weight 1 gram for two-sided sheets), of the additive composition. For comparison purposes, an uncoated paper sheet treated with a composition containing only water by the same procedure was also imaged.

The paper sheets thus prepared were incorporated into a Hewlett-Packard 500-C color ink jet printer containing inks of the following composition:

Cyan: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 30 percent by weight Projet Cyan 1 dye, obtained from ICI, 45.45 percent by weight water.

Magenta: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 2.5 percent by weight Triton Direct Red 227, obtained from Tricon, 72.95 percent by weight water.

Yellow: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 3 percent by weight Hoechst Duasyn Brilliant Yellow SF-GL VP220, obtained from Hoechst, 72.45 percent by weight water.

| Additive                               | Drying Time (minutes) |      |         |        | Optical Density |      |         |        |
|----------------------------------------|-----------------------|------|---------|--------|-----------------|------|---------|--------|
|                                        | black                 | cyan | magenta | yellow | black           | cyan | magenta | yellow |
| none                                   | 10                    | 5    | 5       | 2      | 2.95            | 2.10 | 1.37    | 0.99   |
| D,L-2-amino butyric acid               | 6                     | 3    | 3       | 1      | 2.80            | 2.08 | 1.30    | 0.90   |
| L-arginine hydrochloride               | 6                     | 3    | 3       | 1      | 2.80            | 1.68 | 1.27    | 0.90   |
| D,L-threonine                          | 7                     | 3.5  | 3.5     | 1.5    | 2.40            | 1.81 | 0.90    | 0.77   |
| N-acetyl-D,L-methionine                | 6                     | 3    | 3       | 1.5    | 2.30            | 1.60 | 1.24    | 0.91   |
| β-alanine                              | 7                     | 3    | 3.5     | 2      | 2.80            | 2.20 | 1.25    | 0.90   |
| D,L-alanine                            | 7                     | 3    | 3.5     | 2      | 2.70            | 1.75 | 1.28    | 0.97   |
| D,L-serine                             | 7                     | 3    | 3.5     | 2      | 2.30            | 1.75 | 1.02    | 0.90   |
| D,L-norleucine                         | 7                     | 4    | 3       | 2      | 2.60            | 1.80 | 1.12    | 0.85   |
| L-tartaric acid                        | 6                     | 3    | 3       | 1.5    | 1.60            | 1.68 | 1.45    | 1.01   |
| 2-hydroxy cinnamic acid (methanol)     | 6                     | 3    | 3       | 1.5    | 1.60            | 1.70 | 1.28    | 1.06   |
| 3,4-dihydroxy cinnamic acid (methanol) | 6                     | 3    | 3       | 1.5    | 1.95            | 2.05 | 1.27    | 1.07   |
| 3-hydroxy benzoic acid                 | 7                     | 4    | 3       | 1.5    | 1.60            | 1.47 | 1.20    | 1.07   |

As the results indicate, the drying times of the transparencies containing the additives was generally faster than the drying times of the transparencies containing no additives, while optical densities of images formed on the transparencies containing the additives remained acceptable.

### EXAMPLE III

Paper recording sheets were prepared as follows. Coating compositions containing various additive compositions,

weight Hoechst Duasyn Brilliant Yellow SF-GL VP220, obtained from Hoechst, 72.45 percent by weight water. Images were generated with 100 percent ink coverage. After the image was printed, the paper sheets were each weighed precisely in a precision balance at time zero and periodically after that. The difference in weight was recorded as a function of time, 100 minutes being considered as the maximum time required for most of the volatile ink components to evaporate. (Volatiles were considered to be ink

components such as water and glycols that can evaporate, as compared to components such as dyes, salts, and/or other non-volatile components. Knowing the weight of ink deposited at time zero, the amount of volatiles in the image can be calculated.) After 1000 minutes, the curl values of the paper were measured and are listed in the Table below. The black images were "process black" (i.e., formed by superimposition of cyan, magenta, and yellow images).

| Additive                    | Percent weight-loss of volatiles at various times (minutes) |    |    |    |    |     |          | 1,000 minutes |  |
|-----------------------------|-------------------------------------------------------------|----|----|----|----|-----|----------|---------------|--|
|                             | 5                                                           | 10 | 15 | 30 | 60 | 120 | wt. loss | curl in       |  |
|                             | %                                                           |    |    |    |    |     | mm       |               |  |
| none                        | 32                                                          | 43 | 45 | 48 | 50 | 53  | 65       | 125           |  |
| D,L-2-amino butyric acid    | 39                                                          | 51 | 57 | 60 | 64 | 67  | 72       | 30            |  |
| L-arginine hydrochloride    | 37                                                          | 50 | 54 | 58 | 63 | 66  | 81       | 20            |  |
| D,L-threonine               | 31                                                          | 48 | 55 | 59 | 61 | 65  | 80       | 20            |  |
| N-acetyl-D,L-methionine     | 38                                                          | 50 | 55 | 59 | 64 | 68  | 90       | 10            |  |
| $\beta$ alanine             | 27                                                          | 40 | 45 | 47 | 50 | 54  | 83       | 20            |  |
| L-tartaric acid             | 33                                                          | 49 | 55 | 60 | 64 | 68  | 86       | 15            |  |
| 2-hydroxy-cinnamic acid     | 31                                                          | 47 | 51 | 56 | 58 | 64  | 87       | 15            |  |
| 3-hydroxybenzoic acid       | 37                                                          | 52 | 57 | 61 | 63 | 67  | 94       | 5             |  |
| 3,4-dihydroxy cinnamic acid | 35                                                          | 48 | 52 | 55 | 58 | 64  | 86       | 15            |  |

As the results indicate, the papers containing the additives exhibited higher weight loss values at time 1,000 minutes compared to the paper which had been treated with water alone. In addition, the papers coated with the salts exhibited lower curl values compared to the curl value for the paper treated with water alone.

#### EXAMPLE IV

Paper recording sheets were prepared as follows. Coating compositions containing various salt compositions, each obtained from Aldrich Chemical Co., were prepared by dissolving 50 grams of the salt in 500 milliliters of water in a beaker and stirring for 1 hour at 25° C. The salt solutions thus prepared were then coated onto paper by a dip coating process (both sides coated in one operation) by providing paper base sheets in cut sheet form (8.5×11 inches) in a thickness of 100 microns. Subsequent to air drying at 100° C. for 10 minutes and monitoring the difference in weight prior to and subsequent to coating, the sheets were each coated on each side with 500 milligrams, in a thickness of 5 microns (total coating weight 1 gram for two-sided sheets), of the salt composition. For comparison purposes, an uncoated paper sheet treated with a composition containing only water by the same procedure was also imaged.

The paper sheets thus prepared were incorporated into a Hewlett-Packard 500-C color ink jet printer containing inks of the following composition:

Cyan: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 30 percent by weight Projet Cyan 1 dye, obtained from ICI, 45.45 percent by weight water.

Magenta: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 2.5 percent by weight Triton Direct Red 227, obtained from Tricon, 72.95 percent by weight water.

Yellow: 20 percent by weight ethylene glycol, 2.5 percent by weight benzyl alcohol, 1.9 percent by weight ammonium chloride, 0.1 percent by weight Dowicil 150 biocide, obtained from Dow Chemical Co., Midland, Mich., 0.05 percent by weight polyethylene oxide (molecular weight 18,500), obtained from Union Carbide Co.), 3 percent by weight Hoechst Duasyn Brilliant Yellow SF-GL VP220, obtained from Hoechst, 72.45 percent by weight water. The black images were "process black" (i.e., formed by superimposition of cyan, magenta, and yellow images). The optical densities for the resulting images were as follows:

| Additive                    | Optical Density |      |         |        |
|-----------------------------|-----------------|------|---------|--------|
|                             | black           | cyan | magenta | yellow |
| none                        | 1.08            | 1.18 | 1.03    | 0.80   |
| D,L-2-amino butyric acid    | 1.26            | 1.28 | 1.13    | 0.78   |
| L-arginine hydrochloride    | 1.26            | 1.20 | 1.15    | 0.79   |
| D,L-threonine               | 1.24            | 1.30 | 1.08    | 0.79   |
| N-acetyl-D,L-methionine     | 1.04            | 1.05 | 0.86    | 0.68   |
| $\beta$ -alanine            | 1.20            | 1.10 | 1.15    | 0.80   |
| L-tartaric acid             | 1.02            | 1.00 | 0.84    | 0.70   |
| 2-hydroxycinnamic acid      | 1.03            | 1.16 | 0.70    | 0.65   |
| 3-hydroxybenzoic acid       | 1.03            | 1.15 | 0.71    | 0.66   |
| 3,4-dihydroxy cinnamic acid | 1.01            | 1.11 | 0.69    | 0.68   |

As the results indicate, the papers coated with the additive compositions exhibited acceptable optical densities for all colors.

Other embodiments and modifications of the present invention may occur to those skilled in the art subsequent to a review of the information presented herein; these embodiments and modifications, as well as equivalents thereof, are also included within the scope of this invention.

#### What is claimed is:

1. A recording sheet for receiving printed images which consists essentially of a substrate selected from the group consisting of paper and transparent film and a coating situated on at least one surface of the substrate, said coating consisting essentially of (a) an additive material selected from the group consisting of monomeric amino acids, monomeric hydroxy acids, and mixtures thereof; (b) a quaternary acrylic copolymer latex binder; (c) an optional antistatic agent; (d) an optional biocide; and (e) an optional filler.

2. A recording sheet for receiving printed images which comprises a substrate and a coating situated on at least one surface of the substrate, said coating comprising (a) an additive material selected from the group consisting of monomeric amino acids, monomeric hydroxy acids, and mixtures thereof; and (b) a quaternary acrylic copolymer latex binder.

3. A recording sheet according to claim 2 wherein the additive material is present on the substrate in an amount of from about 1 to about 50 percent by weight of the substrate.

4. A recording sheet according to claim 2 wherein the additive material is present on the substrate in an amount of from about 0.8 to about 40 grams per square meter of the substrate.

5. A recording sheet according to claim 2 wherein the

coating on the recording sheet comprises a polysaccharide binder.

6. A recording sheet according to claim 2 wherein the binder and the additive material are present in relative amounts of from about 10 percent by weight binder and about 90 percent by weight additive material to about 99 percent by weight binder and about 1 percent by weight additive material.

7. A recording sheet according to claim 2 wherein the binder and the additive material are coated onto the substrate in a thickness of from about 1 to about 25 microns.

8. A recording sheet according to claim 2 wherein the substrate is paper.

9. A recording sheet according to claim 2 wherein the substrate is a transparent polymeric material.

10. A recording sheet according to claim 2 wherein the additive is a hydroxy acid.

11. A recording sheet according to claim 2 wherein the additive is of the general formula  $R_1-(CH_2)_n-CH_2-(NHR_2)-COOH$ , wherein  $R_1$  is selected from the group consisting of alkyl, phenyl, hydroxyl, mercaptyl, sulfonic acid, alkyl sulfonic acid, alkyl mercaptyl, phenol, thio, carboxyl, indole, acetamide alkane, 1-alkyl indole, imidazole, aminophenyl, carboxy alkyl, amido alkyl, glutamyl, amino carbonyl, alkyl thio alkyl, amino alkyl, dihydroxy phenyl, vinyl, allyl, amino sulfamoyl, guanidyl alkane, benzyloxy phenyl, S-carbamyl, dicarboxy alkyl, carbobenzyloxy amine, S-trityl, tert-alkoxy carbonyl amine, S-tert alkylthio, S-carboxyalkyl, alkyl sulfoxide alkane, alkyl sulfoxime, hydroxy alkyl, mercaptyl alkyl, thiazolyl, aminalkane, and amine,  $R_2$  is selected from the group consisting of hydrogen, carbobenzyloxy, glycyl, N-tert-butoxy carbonyl, and acetyl, and  $n$  represents the number of repeating units and is a number from 0 to 3.

12. A recording sheet according to claim 2 wherein the additive is selected from the group consisting of alanine; 2-aminobutyric acid; norvaline; norleucine; 2-amino caprylic acid; 2-phenyl glycine; phenyl alanine; homophenyl alanine; serine; cysteine; cysteic acid monohydrate; homocysteic acid; leucine; tyrosine; cystine; aspartic acid; leucenol; acetyl-lysine; tryptophan; trityl-L-cysteine; 1-methyl tryptophan; histidine; 4-amino phenylalanine hydrate; glutamic acid; glutamine; y-glutamylglutamic acid; N-(y-glutamyl) phenylalanine; asparagine; citrulline; ethionine; lysine; lysine hydrate; 3-(3,4-dihydroxy phenyl)-alanine; 2-amino-4 pentanoic acid; 2-amino-4-sulfamoyl butyric acid; arginine; carbobenzyl-tyrosine; carbamyl-cysteine; N- $\epsilon$ (tert-butoxy carbonyl)-lysine; (tert butylthio)-cysteine; y-carboxy glutamic acid; N-carbobenzyloxy-lysine; carboxymethyl-cysteine; methionine; methionine sulfoxide; methionine sulfoxime; homoserine; homocysteine; 3-(2-thiazolyl)-alanine; glycyl glycyl tyrosine dihydrate; glycyl-glutamic acid; threonine; valine; isoleucine; 4-hydroxy phenyl glycine; 3-hydroxynorvaline; N-acetyl-glutamic acid; N-acetyl-methionine; N-a-acetyl-histidine monohydrate; N-acetyl tryptophan; N-acetyl-cysteine; N-acetyl-phenylalanine; N-acetyl-penicillamine; 2-aminobutyric acid;  $\alpha$ -methyl tyrosine; 3-(3,4-dihydroxyphenyl)-2-methyl-alanine sesquihydrate;  $\alpha$ -methylphenylalanine; alanyl-norvaline; alanyl-phenyl alanine; N-(tert-butoxy carbonyl)-isoleucine; N- $\alpha$ -(tert butoxy carbonyl)-lysine; N-(tert-butoxy carbonyl)-phenylalanine; N-(tert-butoxy carbonyl)-serine; N-(tert-butoxy carbonyl)-threonine; N-(tert-butoxy carbonyl)-valine; carbobenzyloxy-alanine; N-carbobenzyloxy-arginine; carbobenzyloxy-asparagine; N-carbobenzyloxy-aspartic acid; carbobenzyloxy-glutamine; N-(carbobenzyloxy)-lysine; N-(carbobenzyloxy)-phenylalanine; carbobenzyloxy-serine; carbobenzyloxy-valine; and mixtures thereof.

13. A recording sheet according to claim 2 wherein the additive is of the general formula  $R_1-(CH_2)_n-CH_2-$

(NHR<sub>2</sub>)—COOH.HX, wherein R<sub>1</sub> is selected from the group consisting of amine, amino alkane, guanidyl alkane, and phenyl alkyl, R<sub>2</sub> is hydrogen or alkyl, n is a number from 0 to 4 and X is an anion.

5 14. A recording sheet according to claim 2 wherein the additive is selected from the group consisting of 2,3-diamino propionic acid monohydrochloride; 2,3-diamino propionic acid monohydrobromide; ornithine hydrochloride; homoarginine hydrochloride; arginine hydrochloride; 2,4-diaminobutyric acid dihydrochloride; lysine monohydrochloride; lysine dihydrochloride;  $\beta$ -methyl-phenyl alanine hydrochloride; 2-methylornithine hydrochloride monohydrate; and mixtures thereof.

10 15. A recording sheet according to claim 2 wherein the additive is of the general formula H<sub>2</sub>N—R—COOH, wherein R is selected from the group consisting of alkane, phenyl, benzyl, alkyl phenyl, phenyl dialkoxy, alkyl cycloalkane, phenol, aminophenyl, diamino phenyl, glycyl, amino benzoyl alkane, amino cycloalkane, methoxy, amino benzophenone, imino phenyl, acetyl alkane, phenyl alkene, phenyl amido alkane, hydroxy alkyl phenyl, dialkyl hydroxy alkyl amino alkane, and benzyl carbonyl.

20 16. A recording sheet according to claim 2 wherein the additive is selected from the group consisting of glycine; glycine hydrochloride;  $\beta$ -alanine; 4-aminobutyric acid; 5-aminovaleric acid; 5-aminovaleric acid hydrochloride; 6-amino caproic acid; 7-aminoheptanoic acid; 8-amino caprylic acid; 11-amino undecanoic acid; 12-amino dodecanoic acid; amino benzoic acid; 3-amino benzoic acid hydrochloride; 4-amino phenyl acetic acid; 4-amino methyl benzoic acid; 5-amino-2-methyl benzoic acid; 2-amino-4,5-dimethoxy benzoic acid; 4-amino methyl cyclohexane carboxylic acid; 5-amino salicylic acid; 3,5-diaminobenzoic acid; 4-aminohippuric acid; glycyl glycine; glycyl glycyl glycyl glycine; N-(4-aminobenzoyl)- $\beta$ -alanine; N-(4-aminobenzoyl)-6-aminocaproic acid; 5-amino isophthalic acid; 1-amino-1-cyclopentane carboxylic acid; 1-amino-1-cyclopropane carboxylic acid hemihydrate; 1-amino-1-cyclopropane carboxylic acid hydrochloride; 4-amino cinnamic acid hydrochloride; succinamic acid; carboxymethoxylamine hemihydrochloride; 2-hydrazino benzoic acid hydrochloride; allantoic acid; 2-aminobenzophenone-2'-carboxylic acid; creatine monohydrate; and mixtures thereof.

30 35 40 45 50 55 60 65 17. A recording sheet according to claim 2 wherein the additive is an imino acid containing —NH and —COOH groups.

18. A recording sheet according to claim 2 wherein the additive is selected from the group consisting of n-trityl glycine; 2-acetamido acrylic acid; 4-acetamido benzoic acid;  $\alpha$ -acetamido cinnamic acid; 6-acetamido hexanoic acid; acetamido acetic acid; N-(2-mercaptopropionyl) glycine; and mixtures thereof.

19. A recording sheet according to claim 2 wherein the additive is of the general formula H<sub>2</sub>N—(R)—SO<sub>3</sub>H, wherein R is selected from the group consisting of alkane, alkylene oxide, phenyl, naphthyl, amino benzene, and acetamido alkane.

20. A recording sheet according to claim 2 wherein the additive is selected from the group consisting of sulfamic acid; amino methane sulfonic acid;  $\alpha$ -2-aminoethane sulfonic acid; 3-amino-1-propane sulfonic acid; 2-amino ethyl hydrogen sulfate; sulfanilic acid; 2-amino-1-naphthalene sulfonic acid; 2,5-diamino benzene sulfonic acid; N-(2-acetamido) 2-amino ethane sulfonic acid; and mixtures thereof.

21. A recording sheet according to claim 2 wherein the additive is of the general formula NH<sub>2</sub>(R)P(O)(OH)<sub>2</sub>, wherein R is selected from the group consisting of alkylene oxide, alkane, and phenyl.

22. A recording sheet according to claim 2 wherein the additive is selected from the group consisting of 2-amino

ethyl dihydrogen phosphate; 2-aminoethyl phosphonic acid; 3-aminopropyl phosphonic acid; 4-amino phenyl phosphonic acid; and mixtures thereof.

23. A recording sheet according to claim 2 wherein the additive is of the general formula HO[R]XH, wherein R is selected from the group consisting of alkane, cycloalkane, phenyl, alkoxy phenyl, dialkoxy phenyl, alkyl phenyl, and phenyl alkene and X is an anion.

24. A recording sheet according to claim 2 wherein the additive is selected from the group consisting of glycolic acid; 10-hydroxydecanoic acid; 12-hydroxydodecanenoic acid; 16-hydroxy hexadecanoic acid; 1-hydroxy-1-cyclopropane carboxylic acid; hydroxy benzoic acid; 3-hydroxy-4-methoxy benzoic acid; 4-hydroxy-3-methoxy benzoic acid; 4-hydroxy-3,5-dimethoxy benzoic acid; 3-hydroxy-4,5-dimethoxy benzoic acid; 2-hydroxy-3-isopropyl-6-methyl benzoic acid; 2-hydroxy-6-isopropyl-3-methyl benzoic acid; hydroxy cinnamic acid; 3-hydroxy-4-methoxy cinnamic acid; 4-hydroxy-3-methoxy cinnamic acid; 3,5-dimethoxy-4-hydroxy cinnamic acid; 2-hydroxyhippuric acid; hydroxy phenyl acetic acid; 4-hydroxy-3-methoxy phenyl acetic acid; 3-(4 hydroxyphenyl) lactic acid hydrate; 4-hydroxyphenyl pyruvic acid; 4-hydroxy benzene sulfonic acid; 3[(1,1-dimethyl-2-hydroxyethyl) amino]-2-hydroxy propane sulfonic acid; and mixtures thereof.

25. A recording sheet according to claim 2 wherein the additive is of the general formula R<sub>1</sub>R<sub>2</sub>(OH)COOH, wherein R<sub>1</sub> and R<sub>2</sub> are each independently selected from the group consisting of alkyl, dialkyl, phenyl, alkoxy, halide, hydroxy, phenyl, dihalide vinyl acrylamide, cycloalkane, and halogenated hydroxyl phenyl.

26. A recording sheet according to claim 2 wherein the additive is selected from the group consisting of lactic acid; 3-hydroxybutyric acid; 2-hydroxyisobutyric acid; 2-ethyl-2-hydroxybutyric acid; 2-hydroxy-3-methyl butyric acid; 2-hydroxy-2-methyl butyric acid; 2-hydroxy caproic acid; hydroxyisocaproic acid; mandelic acid; 4-methoxy mandelic acid; 4-bromo mandelic acid; 3-hydroxy-4-methoxy mandelic acid; 4-hydroxy-3-methoxy mandelic acid; 4-hydroxy mandelic acid monohydrate; 3-chloro-4-hydroxy benzoic acid hemihydrate; 2-hydroxy-3-isopropyl benzoic acid; 3,5-dibromohydroxy benzoic acid; 3,5-dichloro hydroxy benzoic acid; benzilic acid; 2-(4-hydroxy phenoxy) propionic acid;  $\alpha$ -hydroxy hippuric acid; 3,5-diisopropyl salicylic acid; 3-chloro-4-hydroxy phenyl acetic acid; 12-hydroxystearic acid; tropic acid; 2-acrylamido glycolic acid monohydrate; hexahydromandelic acid; and mixtures thereof.

27. A recording sheet according to claim 2 wherein the additive is of the general formula (HO)<sub>2</sub>RCOOH, wherein R is selected from the group consisting of phenyl, acrylic phenyl, phenyl alkyl, phenyl hydroxy, alkyl, naphthyl, alkane amine, diphenyl alkyl, and amino alkyl.

28. A recording sheet according to claim 2 wherein the additive is selected from the group consisting of dihydroxy benzoic acid; 3,4-dihydroxy cinnamic acid; 3,4-dihydroxy hydroxy cinnamic acid; 3,4-dihydroxy mandelic acid; 3,5-dihydroxy-4-methyl benzoic acid hemihydrate; dihydroxy naphthoic acid; dihydroxy phenylacetic acid; bicine; 2,2-bis(hydroxymethyl)propionic acid; 4,4-bis(4-hydroxyphenyl) valeric acid; tris (hydroxymethyl) amino methane succinate; and mixtures thereof.

29. A recording sheet for receiving printed images which comprises a paper substrate and a coating situated on at least one surface of the substrate, said coating comprising (a) an additive material selected from the group consisting of monomeric amino acids, monomeric hydroxy acids, monomeric polycarboxyl compounds, and mixtures thereof; and (b) a quaternary acrylic copolymer latex binder.

30. A recording sheet according to claim 29 wherein the additive is a polycarboxyl compound.

31. A recording sheet according to claim 29 wherein the additive is an aliphatic dicarboxy-functional compound.

32. A recording sheet according to claim 29 wherein the additive is selected from the group consisting of oxalic acid; malonic acid; succinic acid; glutaric acid; adipic acid; pimelic acid; suberic acid; azelaic acid; sebacic acid; undecanedioic acid; 1,10-decane dicarboxylic acid; 1,11-undecane dicarboxylic acid; 1,12,dodecane dicarboxylic acid; hexadecanedioic acid; tetracosane dioic acid; methyl malonic acid; ketomalonic acid monohydrate; ethyl malonic acid; diethyl malonic acid; mercapto succinic acid; methyl succinic acid; malic acid; 2,3-dimethyl succinic acid; citramalic acid; cyclohexyl succinic acid; 2-(carboxymethyl thio) succinic acid; tartaric acid; 2,2-dimethyl glutaric acid; 2,4-dimethyl glutaric acid; 3,3-dimethyl glutaric acid; 2-methyl glutaric acid; 3-methyl glutaric acid; 3,3-tetramethylene glutaric acid; 3-phenyl glutaric acid; 2-ketoglutamic acid; 3-ketoglutamic acid; 3-methyl adipic acid; 2,6-diamino pimelic acid; 4-ketopimelic acid; mucic acid; 3-methylene cyclopropane-trans-1,2-dicarboxylic acid; 1,1-cyclobutane dicarboxylic acid; cyclohexane dicarboxylic acid; imino diacetic acid; (N-(2-acetamido) imino diacetic acid); methyl iminodiacetic acid; diglycolic acid; 1,1-cyclohexane diacetic acid; fumaric acid; maleic acid; glutaconic acid; 2-dodecenedioic acid; mesaconic acid; citraconic acid; dihydroxy fumaric acid hydrate; trans, trans-1,3-butadiene-1,4-dicarboxylic acid; and mixtures thereof.

33. A recording sheet according to claim 29 wherein the additive is an aromatic dicarboxy-functional compound.

34. A recording sheet according to claim 29 wherein the additive is selected from the group consisting of homophthalic acid; terephthalic acid; phthalic acid; 4-methyl phthalic acid; chelidonic acid monohydrate; chelidamic acid monohydrate; cis-5-norbornene-endo-2,3-dicarboxylic acid; 1,4-naphthalene dicarboxylic acid; 2,3-naphthalene dicarboxylic acid; 2,6-naphthalene dicarboxylic acid; 4-carboxy phenoxy acetic acid; 2,5-dihydroxy-1,4-benzene diacetic acid; pamoic acid; 4-(4-(2-carboxybenzoyl) phenyl) butyric acid; 1,4-phenylene diacrylic acid; 2-carboxy cinnamic acid;  $\alpha$ -glutamyl-L-cysteinyl glycine; isocitriclactone (2-oxotetrahydrofuran-4,5-dicarboxylic acid; N-(2-hydroxyethyl) iminodiacetic acid); dipivaloyl-tartaric acid; cyclohexyl succinic acid; phenyl diacetic acid; and mixtures thereof.

35. A recording sheet according to claim 29 wherein the additive is a polycarboxyl compound having more than 2-COOH groups.

36. A recording sheet according to claim 29 wherein the additive is selected from the group consisting of 1,3,5-cyclohexane tricarboxylic acid; citric acid monohydrate; 1,2,3-propene tricarboxylic acid; 1,2,3-propane tricarboxylic acid;  $\beta$ -methyl tricarballylic acid; 1,2,3,4-cyclobutane tetracarboxylic acid; 1,2-diaminocyclohexane-N,N,N',N'-tetraacetic acid hydrate; 1,6-diaminohexane-N,N,N',N'-tetraacetic acid hydrate; 1,2,4,5-benzene tetracarboxylic acid; 1,4,5,8-naphthalene tetracarboxylic acid hydrate; penta diethylene triamine penta acetic acid; mellitic acid; agaric acid; 1-2-diamino propane-N,N,N',N'-tetra acetic acid; ethylene diamine tetraacetic acid; 2-(carboxymethylthio) succinic acid; N-(2-hydroxyethyl) ethylene diamine triacetic acid; N,N'-bis(2-carboxyethyl)-N,N'-ethylene di glycine trihydrate; tetrahydrofuran-2,3,4,5-tetracarboxylic acid; and mixtures thereof.